

Jan. 12, 1965

A. ROY ET AL

3,165,400

CASTABLE HEAT RESISTING IRON ALLOY

Filed June 27, 1961

8 Sheets-Sheet 1



FIG. 1.

BY

INVENTORS.  
Amédée Roy  
Walter E. Tominy  
Harriss & Harris  
ATTORNEYS.

Jan. 12, 1965

A. ROY ET AL.

**3,165,400**

## CASTABLE HEAT RESISTING IRON ALLOY

Filed June 27, 1961

8 Sheets-Sheet 2



FI [REDACTED] .2 .

BY

INVENTORS.  
Amédée Roy  
Walter E. Tominy  
Harness & Harris  
ATTORNEYS.

Jan. 12, 1965

A. ROY ET AL

3,165,400

CASTABLE HEAT RESISTING IRON ALLOY

Filed June 27, 1961

8 Sheets-Sheet 3



FIG. 3.

BY

INVENTORS.  
Amedee E. Roy  
Walter E. Tonning  
Harnois & Harnois  
ATTORNEYS.

Jan. 12, 1965

A. ROY ET AL

3,165,400

CASTABLE HEAT RESISTING IRON ALLOY

Filed June 27, 1961

8 Sheets-Sheet 4



FIG. 4.

BY

INVENTORS  
Ameliee Roy  
Walter E. Tominy  
Harnois & Harnois  
ATTORNEYS.

Jan. 12, 1965

A. ROY ET AL

3,165,400

CASTABLE HEAT RESISTING IRON ALLOY

Filed June 27, 1961

8 Sheets-Sheet 5



BY

INVENTORS.  
Amedee Roy  
Walter E. Torrey  
Harness & Harris  
ATTORNEYS.

Jan. 12, 1965

A. ROY ETAL

3,165,400

CASTABLE HEAT RESISTING IRON ALLOY

Filed June 27, 1961

8 Sheets-Sheet 6



FIG. 6.

BY

INVENTORS.  
Amedee Roy,  
Walter E. Tominy,  
Harniss & Harris  
ATTORNEYS.

Jan. 12, 1965

A. ROY ET AL

3,165,400

CASTABLE HEAT RESISTING IRON ALLOY

Filed June 27, 1961

8 Sheets-Sheet 7



FIG. 7.

BY

INVENTORS  
Amedee Roy  
Walter E. Tommy  
Harnois & Harris  
ATTORNEYS

Jan. 12, 1965

A. ROY ET AL

**3,165,400**

## CASTABLE HEAT RESISTING IRON ALLOY

Filed June 27, 1961

8 Sheets-Sheet 8



INVENTORS.  
Amedee Roy.  
Walter E. Sommity.  
BY  
Harvey & Harris.

Harness & Harris

ATTORNEYS.

## 1

3,165,400

## CASTABLE HEAT RESISTING IRON ALLOY

Amedee Roy, Ferndale, and Walter E. Jominy, Detroit, Mich., assignors to Chrysler Corporation, Highland Park, Mich., a corporation of Delaware

Filed June 27, 1961, Ser. No. 119,902

21 Claims. (Cl. 75—126)

This invention relates to iron base alloys austenitic at room and operating temperatures and possessing high stress rupture properties at temperatures above 1200° F. and up to 1500° F. and in excess thereof even up to 1700° F. without the use of substantial amounts of the strategic elements nickel (Ni) and cobalt (Co) and even in the substantial absence of one or both. It especially concerns alloys of this character possessing in high temperature service stainless properties for resisting oxidation and providing substantial strength and load carrying ability and great resistance to creep and deterioration by heat. It also particularly refers to iron base alloys of the aforesaid character useful for producing cast articles of complicated shapes for instance, by precision casting processes. Moreover, it has specific reference to alloys of the foregoing character and properties which are relatively high in carbon content and which are weldable by known procedures.

The mass production of many mechanical parts depends upon the development of low cost, non-strategic alloys which provide adequate strength and oxidation resistance at the high temperature service conditions at which such parts are to operate. Typical examples are furnace and turbine parts, internal combustion engine valve parts and heat treat fixtures. Iron base alloys high in carbon and ferritic at room temperatures are not suitable for applications such as these where temperatures in the range of 1200° F. to 1700° F. and relatively high stress conditions are encountered. Moreover, they are either not suitable for welding or may only be welded with substantial difficulty.

Cobalt base alloys rich in nickel, for example Stellite alloy HS31 and nickel base alloys usually referred to as highly alloyed "super alloys," have been proposed for meeting some of the properties required for such rigorous service but these high strategic element alloys cannot at present be considered for most mass produced structures because of their high cost and the high content of strategic elements such as cobalt and/or nickel they necessarily contain. Moreover, attempts made to produce substitute castable alloys low in the strategically scarce elements cobalt and/or nickel, have not insofar as we are aware, produced any having the foregoing physical properties required at temperature between 1200° to 1700° F. nor have such attempts produced any alloy approaching the service life possible with available "super alloys" predominant in cobalt and nickel. Even heat treatment of such alloys has not developed satisfactory high temperature mechanical properties.

There is a need not only for satisfactory iron base alloys low in strategic elements but also a great demand for weldable alloys of such character suitable for producing articles of complicated shape, for instance, turbine blades and nozzle blocks by precision casting methods.

A disadvantage of many alloys high in strategically scarce elements is the necessity in many cases of employing special high temperature heat treatments in order to develop their high temperature properties. This is very costly. Moreover, even with these heat treatments we are not aware that any ferrous base alloy for the above

## 2

application has been commercially available providing a 100 hour rupture strength of at least 20,000 p.s.i.

The present invention aims to solve the aforesaid problems and provide suitable iron base alloys not requiring large amounts of any strategic elements especially cobalt and/or nickel and capable of providing the required high physical and service properties. It is based upon the discovery that iron base alloys are structure sensitive at high temperatures and that obtaining desired room temperature and high temperature properties aforesaid is dependent upon the proper proportioning in low critical amount of certain austenite forming elements especially carbon and nickel and NaCl-type carbide formers in association with other essential elements of the composition.

More particularly it is based upon the discovery that improved room temperature and high temperature properties are imparted to iron base alloys for casting into complex shapes, by the presence of substantial amounts of carbon and by the presence of multiple and controlled additions of the NaCl-type of cubic carbide-forming elements in a stable and balanced austenitic composition containing critical amounts of carbon and nickel and that the NaCl-type of cubic carbides of a selected group of elements are found to possess a very high degree of stability at elevated temperatures conducive to the making of low nickel, cast austenitic stainless steels which may be cobalt free, with outstanding stress rupture properties at high temperatures of 1500° F. and even higher. In particular cases by a proper combination of critical amounts of certain carbide forming elements with nitrogen, the alloy may even be made nickel free.

A fundamental object is therefore to provide new and improved heat resisting castable iron base alloys austenitic at room temperatures, relatively high in carbon, low in strategic element content especially nickel and cobalt, and which may be completely free of one or even both of these elements, and that are characterized by stability, strength and oxidation and creep resistance in high temperature service.

Another object is to provide new and improved high strength iron base castable alloys austenitic at room temperature and low in strategic element content especially nickel and cobalt that possess the requisite casting properties demanded by precision casting procedures.

A further object is to provide new and improved high temperature iron base alloys as in the preceding objects which do not require special heat treatment to develop vastly improved high temperature properties but which may in certain cases by still further improved thereby.

A particular object is to provide high carbon stainless iron base alloys austenitic at room temperature and low in strategic elements which possess at high temperatures of 1500° F. properties comparable or superior to those attained by so-called "super alloys" high in one or more of the strategic elements nickel and/or cobalt.

A specific object is to provide a heat resisting stainless iron base alloy containing in the order of 60% and more iron by weight and which may be low in nickel and free of cobalt, which alloy is austenitic at room temperature, suitable for producing cast turbine blades and the like, and will provide articles of this character with adequate ductility and strength at room temperature and the ability to resist creep, oxidation and scaling at temperatures of 1500° F. and greater encountered in the type of service to which such articles are subject.

Another specific object is to provide an alloy composition comprising a wholly austenitic iron, solid solution matrix relatively high in carbon content in which in-

soluble primary and lamellar-type carbides are embedded and which contains dot-type carbides and angular intermetallic compounds randomly distributed in the matrix and semi-continuously in the grain boundaries.

A further object is to produce an iron base alloy composition relatively high in carbon content providing a matrix having a stable austenitic face-centered cubic structure (F.C.C.) as lean as possible in the requisite non-strengthening substituent type austenitic forming elements in order to facilitate the addition of optimum amounts of matrix strengtheners without overstraining the iron lattice of the structure at both room and elevated temperatures.

A particular object is to produce an iron base alloy composition low in strategic elements and relatively high in carbon that has good physical properties at high temperatures and that is readily weldable.

It is also an object to provide an iron base alloy containing a relatively high optimum concentration of carbon stoichiometrically balanced with NaCl-type of carbide formers to prevent on one hand the formation of undesirable carbides and on the other hand, to prevent an excess of lattice straining elements.

It is a further object to provide an alloy matrix whose composition comprises an iron base alloy relatively high in carbon content containing dissolved and combined nitrogen, in controlled concentration and balanced to the total amount of nitride formers such as chromium, manganese and columbium present therein.

A further specific object is to provide a low cost alloy metal having optimum load-carrying ability and creep resistance at high temperatures between 1200° F. to 1700° F. which comprises a stable iron base castable alloy austenitic at room and operating temperatures including as essential ingredients, predetermined relatively small amounts of austenite forming elements from the group consisting of carbon, nickel and manganese, such consisting at least of carbon in substantial amount and of nickel and predetermined relatively small amounts of a plurality of carbide and/or nitride forming elements including molybdenum, tungsten, and at least one selected from the group consisting of columbium, tantalum, titanium, and vanadium, preferably columbium and/or tantalum, and better still, columbium which has been found to possess especially good carbide and nitride forming properties.

Another object is to provide an iron base alloy as in the preceding objects that includes free or uncombined chromium in amount sufficient to render the metal stainless in character and oxidation resistant at high temperatures between 1200° F. to 1800° F.

An additional object is to provide an iron base alloy having high stress resistance properties and a face-centered cubic solid solution structure stable at room temperature that includes in addition to chromium and critical amounts of carbon, small predetermined amounts of nickel and in particular instances, nickel and/or manganese for stabilizing the austenitic structure by substitution for iron, and other strengthening elements such as nitrogen, molybdenum, tungsten, columbium, tantalum, titanium, and vanadium in predetermined combinations in solid solution or as a precipitate for the purpose of matrix strengthening without overstraining the iron lattice.

Other objects and advantages of our invention will appear from the following additional description and from the drawings wherein:

FIGURE 1 represents a photomicrograph (1000 $\times$ ) of a cast alloy No. 124 containing 0.38% carbon, which alloy is not within the scope of our invention and which was taken from a  $\frac{1}{4}$ " diameter test bar heated for about 100 hours at 1500° F. The alloy is austenitic. The light colored area indicated by letter A represents the austenitic phase, the black areas indicated by the letters B represent eutectic (ledeburite) phases randomly dispersed throughout the structure. The alloy is character-

ized by the absence of secondary precipitates except for a few localized secondary carbides at C precipitated from the austenitic matrix.

FIGURE 2 represents a photomicrograph (1000 $\times$ ) of a cast alloy No. 123 containing 0.54% carbon, which alloy is also not within the scope of our invention and which was taken from a  $\frac{1}{4}$ " diameter test bar heated for about 100 hours at 1500° F. The alloy is austenitic. The light colored area indicated by the letter A signifies the austenitic phase, the letters B represent the eutectic (ledeburite) phases randomly dispersed throughout the structure, and the letter C refers to dot-like secondary carbides randomly dispersed within the matrix and locally concentrated toward the eutectic phases.

FIGURE 3 represents a photomicrograph (1000 $\times$ ) of a cast alloy similar to No. 123 but containing 0.7% carbon taken from a  $\frac{1}{4}$ " diameter test bar heated for about 100 hours at 1500° F. The alloy is austenitic. It is similar in general structural characteristics to the alloy of FIGURE 2 but differs in that there is a greater amount of randomly dispersed eutectic phases B in the austenitic phase A. Also, there is a greater concentration of dot-like secondary carbides C within the matrix.

FIGURE 4 represents a photomicrograph (1000 $\times$ ) of a cast alloy No. 120 of our invention containing 0.83% carbon taken from a  $\frac{1}{4}$ " diameter test bar heated for about 100 hours at 1500° F. The alloy is austenitic. The structure is significantly different from those of FIGURES 1 to 3, inclusive, in that the eutectic (ledeburite) phases B form a distinctive well defined network surrounding the austenitic phases A imbedding dot-like secondary carbides C which are heavily concentrated toward the network and more uniformly distributed throughout the austenitic phase A than in the previously described microstructures.

FIGURE 5 represents a photomicrograph (1000 $\times$ ) of a cast alloy No. 6 of our invention containing 1.05% carbon taken from a  $\frac{1}{4}$ " diameter test bar heated for about 100 hours at 1500° F. The alloy is austenitic and is of the general character of that of FIGURE 4, but is notable by its heavier well defined network of the eutectic (ledeburite) phases B outlining the austenitic matrix areas A and heavier concentrates of fine secondary carbide precipitates C within the austenitic phase.

FIGURES 6 and 7 represent photomicrographs (1000 $\times$ ) of cast alloys Nos. 105 and 66, respectively, containing 1.2% and 1.41% carbon, respectively, taken from  $\frac{1}{4}$ " diameter test bars heated for about 100 hours at 1500° F. The alloys are similar in general structure to that of FIGURES 4 and 5, but are characterized by the presence of increasing density in the eutectic (ledeburite) network.

FIGURE 8 is a graph showing the effect of varying the carbon content of a basic alloy composition such as alloy No. 6 on the 100 hour stress rupture strength at 1500° F. and room temperature tensile test percent elongation.

The above photomicrographs of FIGURES 1 to 7, inclusive, are those respectively taken of a representative portion of the longitudinally cut surface of longitudinally sectional  $\frac{1}{4}$ " diameter temperature treated test bars of the alloys represented after such cut surfaces had been mechanically polished and then electrolytically etched for 15 to 25 seconds in a 10% oxalic aqueous acid solution at a current density of between 0.25 to 0.5 ampere per square inch.

The term "austenitic alloy" as used herein is intended to mean a face centered cubic (F.C.C.) solid solution of iron which is stabilized by the addition of austenite forming elements such as nickel, nitrogen, manganese, and carbon and which is austenitic at room and service temperatures and will not transform to a body centered cubic (B.C.C.) solid solution or ferritic state upon cooling slowly to room temperature after service at high temperature.

As mentioned briefly above, our invention is, among

other things, based upon the discovery that stable austenitic ferrous alloys, especially those having stainless qualities and other combinations of physical properties described above, may be obtained by combining small critical quantities of certain austenite forming elements of the group nickel (Ni), manganese (Mn), carbon (C), and nitrogen (N) of which carbon is essential and is relatively high and nickel is essential except in the case of particular combinations of manganese and sometimes nitrogen, with an iron base material and with small critical quantities of a plurality of certain NaCl-type carbide formers of the group molybdenum (Mo), tungsten (W), columbium (Cb), tantalum (Ta), titanium (Ti), and vanadium (V), to produce a stable austenitic matrix at room and operating temperatures and to provide a balanced alloy with outstanding combinations of room and elevated temperature properties. Such features make it possible to obtain iron base alloys possessing properties comparable or superior to alloys high in nickel and/or cobalt.

The new alloys are low cost, investment-castable, weldable austenitic stainless steels preferably containing about 60% and more iron by weight and having a 100-hour stress-rupture strength at 1500° F. of the order of 22,000-28,000 p.s.i. and even higher in the as cast condition. These alloys also possess high strength at room temperature and are more readily weldable than the known HS31 and HS21 alloys.

In general the preferred stable austenitic compositions of our invention of the aforementioned character having one or more of the described properties, and which may be free of or contain small amounts of cobalt will preferably contain in addition to iron as essential ingredients the elements carbon, silicon, nickel, manganese, nitrogen, chromium, molybdenum, tungsten, and columbium and/or tantalum preferably columbium.

The amounts of each by weight percent will depend upon the specific properties desired and may be broadly expressed by a composition containing as essential ingredients at least about 0.8% and up to about 1.25% carbon, about 2 to 8% nickel, about 1 to 15% manganese, about 12 to 35% chromium and a plurality of molybdenum, tungsten and metal from the group columbium and tantalum in amount not greater than about 12%, preferably not more than about 9% with the molybdenum when used within about 0.1 to 9%, tungsten when used within about 0.1 to 10% and columbium and/or tantalum when used within about 0.1 to 5%. In no case should the combined nickel and manganese exceed about 15%. The composition will also desirably include silicon in amount between 0 to about 2.5% preferably at least about 0.3% and nitrogen in amount between 0 to about 0.6%, the latter being especially significant when the nickel is at the 2% level or less and especially when the carbide forming elements are above a total of 3% in the latter cases nitrogen additions of 0.05 to 0.6% and preferably between about 0.05 to 0.3% are a decided advantage. The alloy may also optionally include cobalt in amount between 0 to about 8% in which case the combined total of nickel, manganese and cobalt should not exceed about 15%. The remainder of the composition will essentially be iron which should constitute at least 40% and may be as high as 75% of the alloy. Compositions within the foregoing range of ingredients will provide alloys having the physical properties of at least about 2% elongation with a tensile strength of at least about 85,000 p.s.i. at room temperature, a hot tensile strength at 1500° F. of at least about 40,000 p.s.i. with less than 35% elongation, and a 100 hour rupture life at 1500° F. of at least about 20,000 p.s.i. believed a desirable minimum for commercial applications.

In certain special cases where something less than 2% elongation is acceptable the upper limit of carbon may be increased to about 1.6%. Moreover, vastly improved physical properties providing 100 hour rupture strengths at 1500° F. of above 22,000 p.s.i. and in the order of

24,000 to 28,000 p.s.i. will be obtained when the carbon content is above 0.9% and for optimum results above a minimum of about 1% and up to about 1.1%. Furthermore, in certain instances when the optimum properties provided by the presence of both nickel and manganese are not required, manganese may be entirely omitted in the above compositions or used in amount less than 1% providing at least about 2% nickel be used. Moreover, nickel may be used in amount less than 2% providing that between about 5 to 10% manganese is included and at least about 10% where the nickel content is zero. The amount of manganese in these cases may be reduced to as low as about 2% if some nitrogen preferably at least about 0.3% is provided.

In place of a portion of the iron content in the above compositions and while maintaining at least a 40% concentration there may also be included in the alloy in certain cases for the special advantages hereinafter noted they may supply, certain other elements, for example up to 5% titanium, up to 5% vanadium, up to 1% boron, up to 0.2% phosphorous and such incidental elements as zirconium, aluminum, and magnesium which may be present as a result of master addition alloys employed during processing, reactions between melt and crucible, deoxidizers, degasifiers and purifiers which do not deleteriously effect the properties of the alloy (the total of which incidental elements will not ordinarily exceed about 1%). Hence the expression "the balance" or "the remainder" whenever used in reference to the composition shall be construed to include any of these additions and contaminating elements. To avoid the inclusion of uncontrolled amounts of contaminating elements which may cause some degradation of physical properties it is preferred that starting ingredients be employed whose compositions are known both as to primary and trace elements.

We have particularly discovered that a combination preferably in substantially stoichiometrically balanced amounts of the NaCl-type of carbide formers, molybdenum, tungsten and at least one from the group consisting of columbium and tantalum, preferably columbium which is found to be superior to tantalum in the properties given to the matrix, in relatively small properly proportioned quantities, in a suitable austenitic matrix containing between above about 0.9 and up to 1.1% carbon and other essential ingredients within the limits previously stated will produce low cost alloys possessing exceptionally high resistance to stresses at high temperature. Based upon experimentation, we preferably maintain the amount of molybdenum within the range of about 0.2% to 7.0% tungsten within about 0.2% to 6% and columbium and/or tantalum alone or combined in either case within the range of about 0.2% to 4.0% and with a total of molybdenum, tungsten, columbium and/or tantalum not exceeding about 9% by weight.

Thus for making lowest cost precision castable alloys having a tensile strength of at least 85,000 p.s.i. at room temperature and at least about 2% elongation, a hot strength of at least 40,000 p.s.i. at 1500° F. with less than 35% elongation and a 100 hour rupture strength at 1500° F. of at least 24,000 p.s.i., believed adequate for uses which have heretofore required high nickel or cobalt alloys, the alloy compositions will contain as essential ingredients in critical amounts about 0.9% to 1.1% carbon, preferably above a minimum in the order of 1.0%, 0.1% to 2% silicon, 12% to 25% chromium, 0.2% to 7% molybdenum, 0.2% to 6% tungsten, 0.2% to 4% columbium and/or tantalum, with a total of molybdenum, tungsten, columbium, and/or tantalum not exceeding about 9%, 2.0% to 8% nickel, 0% to 9% manganese with a total combined maximum content of nickel and manganese in the order of 11%, the balance being essentially iron in amount at least about 40%, preferably 60%, and as high as about 75%. In place of part of the iron and while maintaining at least a 60% iron concentration, there may be also included 0% to

3% titanium, 0% to 3% vanadium, 0% to 0.4% boron, 0% to 0.2% phosphorous, 0% to 0.6% nitrogen and the incidentals mentioned above. Cobalt may be optionally added in amount between 0% to 8% in which event the combined total of nickel, manganese and cobalt should not exceed 15%. Moreover, best results are obtainable when the molybdenum, tungsten, and columbium (or tantalum) are used in substantially equal amounts in the range of about 1% to 2% of each. Equal amounts are likewise preferred above the 2% level. Where the molybdenum, tungsten, columbium (or substituent tantalum) are used in substantially equal amounts at levels from about 2% to 4%, nitrogen in amount between 0.05 to 0.6% is found beneficial to the mechanical properties of the alloy and should preferably be included.

Carbon must always be present in the new alloys, it not only being an austenite former but more particularly combining with the NaCl-type of cubic carbide formers molybdenum, tungsten, columbium, tantalum, titanium, and vanadium with which it must be balanced, preferably stoichiometrically to form among other carbides the simple carbides MoC, WC, CbC, TaC, TiC, VC and complex carbides of these with chromium such as the  $M_{23}C_6$  types. For optimum creep-rupture strength, the iron base alloys of our invention require a carbon content above an amount in the order of about 1% and in the range 0.9 to 1.1%, preferably stoichiometrically balanced with the addition of these strengthening elements.

Variations in carbon content not only profoundly affect the stress rupture strength at 1500° F., the room temperature percent elongation and the stress rupture elongation at 1500° F. of alloys having compositions otherwise within the foregoing ranges of ingredients, but are found to produce marked changes at certain levels in the microstructure of the alloys. Thus we have discovered that the 100 hour rupture life at 1500° F. peaks at about 1% carbon, that the room temperature percent elongation surprisingly does not follow the sharp downturn expected with increasing carbon content but levels out at about 0.8% carbon and extends over a range of carbon between 0.8% to 1.25% carbon and provides satisfactory ductility in this range, and that the stress rupture elongation at 1500° F. similarly undergoes a surprising change at 0.8% carbon reversing the expected continued downturn with increasing carbon content and is in a safe preferred range of between 5 and 25% elongation. Moreover, it is found that alloys with a carbon content below 0.8% carbon have an appreciable change in microstructure from those in the range of 0.8% to 1.4% carbon and that below about 0.5% carbon there is a drastic change occurring in microstructure. These distinctions in structure and physical properties will be readily evident from the photomicrographs of FIGURES 1 to 7, inclusive, and the above descriptions thereof, and from the graphs of physical properties in FIGURE 8 of a typical base composition with varying carbon content. From this data it should be apparent that alloys below 0.8% carbon have substantially weaker physical properties and that increases in carbon above about 1.25% does not appear to strengthen the alloys to any appreciable extent at least to be of practical value, but renders the cold ductility of the alloys in most cases inadequate. Hence carbon in the range 0.8% to 1.25% is preferred and for optimum results carbon above an amount in the order of about 1% and in the range 0.9% to 1.1% gives best results.

A further feature of our invention is the critical proportioning of the NaCl type carbide formers to the carbon content of the alloy. The resulting complex carbide phases are highly resistant to spheroidization at elevated temperatures and give to the alloy matrix great physical stability under load at high service temperatures. The elevated temperature properties, creep resistance and heat resistance of the alloys is decisively influenced by the character and amount of these carbide

forming elements present in the alloy. Multiple additions of carbide forming elements in optimum amounts impart much greater creep resistance than any single addition thereof in comparable or even greater amount.

Thus the most potent strengthening elements are found to be tungsten, molybdenum and columbium. We have discovered that optimum high temperature properties are achieved through the use of triple combinations of these NaCl-type of cubic carbide-forming elements in a suitable basic composition containing the other essential elements referred to above and within the limits stated, for example in a basic composition containing about 20% chromium, about 5% nickel and about 5% manganese.

A combination of a substantially 1:1:1 ratio of tungsten, molybdenum, and columbium in the basic alloys achieves the best properties. For instance, an alloy, as in example No. 6 in the tables, containing approximately 1% each by weight of W, Mo, and Cb, about 1% C, about 20% Cr, about 5% Ni, about 4.5% Mn, and about 1% Si displayed a 100 hour rupture strength of 27,000 p.s.i. at 1500° F., a cold tensile ductility of 4% elongation, good oxidation resistance up to 1800° F. and was readily weldable. The tables show examples using other equal amounts of these strengthening elements. See for example, alloys 303, 14, 15, 4, and 7 from which it will be evident that the 100 hour stress rupture strength is optimum in the range of 0.1% to 2% increasing with quantities up to 1% and decreasing with increasing quantities above 2%. A maximum of 4% of each is preferred as an upper limit.

Simultaneous variations in the amount of W, Mo, and Cb at the 6% to 10% levels depressed the stress rupture properties of the basic alloy compositions. However, large additions of molybdenum using smaller amounts of tungsten and columbium within the 12% total improved the hot tensile strength while high columbium additions had the reverse effect. Large additions of tungsten acted similarly to the molybdenum.

Titanium and vanadium are also possible additives in lieu of or as a replacement of part of the columbium and tantalum, used and preferably within the limits set forth for these latter elements. Titanium and vanadium are not especially recommended since experiments seem to indicate that they are prone to permit more severe oxidation of the matrix during service than where columbium or tantalum are used without them and thus tend to lower the ultimate stress value. Titanium and vanadium are also not as suitable as columbium and tantalum from the standpoint of room temperature ductility and alloy castability. They tend to produce lower ductility and in certain cases affect mold reaction during investment-type casting, resulting in castings with surfaces not as smooth as those obtained when columbium or tantalum are employed from the stated group.

As previously noted, an essential feature of our invention is that the alloy be austenitic. For this purpose the nickel content in the absence of manganese, or nitrogen or cobalt should not be less than about 2%. It is also desired and important that the austenite formers others than carbon, i.e., nickel, manganese, nitrogen, and cobalt should be adjusted to obtain in conjunction with the essential carbon content an austenitic composition that is not only stable but of optimum high temperature properties, a condition attained when the non-strengthening austenite formers (nickel and cobalt) are not present in excessive amount, and the austenite formers carbon, manganese, nitrogen which form strengthening carbides and nitrides are optimum in amount. Hence the amount of nickel required will decrease with increasing amount of austenite formers carbon, manganese, and nitrogen used. The amount of nickel needed to contribute to stability will also vary with the character and amount of the other essential ingredients of the alloys especially all of the ferrite formers chromium, molybdenum, tung-

sten, columbium, tantalum, and silicon. For the amounts of carbon used in our alloys, an amount of nickel between about 2% to 8% will produce optimum properties. These properties are far superior to those attainable with high concentrations of nickel and lower concentrations of carbon. In fact, these properties approach, and even surpass those of the known super alloys as will hereinafter be evident.

Where cost is not material and optimum high temperature properties are not essential, higher nickel concentrations than 8% may be used in conjunction with the other essential ingredients of the alloy to obtain some improvement in oxidation resistance. Amounts of nickel in excess of 20%, for instance up to 35%, will not only adversely affect room temperature and high temperature stress rupture properties but will also decrease the solubility of nitrogen in the alloy to a point where additions of the latter in amount to provide desirable properties thereby in the alloy will be inhibited. Moreover, such may require a reduction in the minimum amount of iron desired in the alloy and for many applications will make cost prohibitive. Hence, nickel in amounts up to about 8% is preferred and amounts in excess of 20% not generally advocated.

Manganese is also preferably employed in producing the alloys of our invention and in amounts up to about 15% by weight. Amounts between 0% to 7% are preferred as in this range, the manganese in addition to being a nitride former, is also a relatively strong austenitizer and is somewhat effective in improving the castability of the alloy. About 5% gives best results. Replacing nickel with manganese or raising the manganese at the standard nickel level of about 2% to 8% will produce higher tensile strengths at 1500° F. with no apparent change in rupture strength. The cold tensile ductility may in certain cases, however, be somewhat below optimum.

The addition of nitrogen to the alloy composition is sometimes advantageous. It may be used as a substitute for other austenite formers and when included tends to stabilize the austenite composition. Moreover, nitrogen combines to some extent with the chromium of the alloy and to a smaller extent with the manganese when the latter is present to form nitrides and with columbium to form carbonitrides. In certain alloys the production of precipitation hardening nitrides is believed to be partly responsible for the improved high temperature strength and the high temperature service life of the alloys of our invention. Many of the better alloys produced by our invention will contain optimum amounts of nitrogen. The total amount of nitrogen that can be held in stable combination in the alloys depends upon the nickel, chromium, columbium and manganese content of the alloy. Nickel as previously noted when used in large amounts, reduces the amount of nitrogen that may be present. Chromium and manganese have the opposite effect. When nitrogen and manganese are used in optimum amounts as in alloys 86a-86d for example, it is even possible to obtain an alloy with excellent properties without using any nickel or cobalt. Too high uncombined nitrogen is believed to be detrimental to the high temperature properties of the alloys since higher porosity of the casting is often observed where too much nitrogen is in the mass. This element will preferably be used in amounts not exceeding about 0.6%.

As previously described, the alloys of our invention are preferably endowed with stainless properties. For this purpose chromium is an essential ingredient; a minimum of about 8% and a maximum of 35% is preferred. We have found that amounts between about 12% to 25% usually provide adequate oxidation and corrosion resistance at high temperatures up to about 1800° F.

Silicon usually occurs as an impurity in the alloys of our invention in amounts up to about 0.5% to 0.7% (see tables). This is especially the case where commercial grades of master alloys are used in their preparation. The

effect of silicon is threefold. First it influences the solidification characteristics of the alloy such as fluidity, castability, and weldability. Secondly, it influences the physical properties at both room and elevated temperatures. Thirdly it is a strong deoxidizer.

Thus with regard to weldability, the presence of at least 0.4% silicon in the stable austenitic alloys of our invention, lean in austenite formers, provides a balanced structure with the embrittling carbide forming elements when the carbon content is above 0.8% whereby there is present in the network a relatively small amount of dispersed ferrite. This facilitates the making of a ductile weld.

It is known that castable iron alloys with over 0.8% carbon are not readily weldable. Also that most "super alloys" are so brittle with even much less carbon that they must not only be preheated to prevent cracking during welding but must also be postheated to relieve stresses produced during welding, to avoid after cracking. The alloys of our invention avoid these steps and conditions so long as the amount of silicon present remains under about 2.0%. Silicon above this amount will embrittle the alloy particularly at room temperature and reduce the stress rupture strength at 1500° F. Moreover, silicon is a very effective deoxidizer and as such not only influences the ductility of the alloy as prepared, but also the character of any weld. Furthermore, it improves resistance of the alloy to oxidation at elevated temperatures.

The iron base alloys of our invention may also include certain other specific elements such as phosphorous, boron and sulphur. Thus as previously indicated, boron may be added in amounts from 0 to 1% to improve the high temperature strength of the alloy. It is found, however, that boron in amounts above 0.04% will cause a decrease in room temperature ductility. Phosphorous when added in amounts up to about 0.1% renders the alloy susceptible to heat treatment with corresponding improved hot strength. Increasing amounts of phosphorous tends to decrease the ductility of the resulting alloy.

Although the alloys of our invention are characterized as being cobalt-free, additions of cobalt are found in some cases to have a beneficial influence on the castability and the high temperature properties of the alloys and where some additional cost is warranted between 0% to 15% of this element may be included in the alloy composition. However, it is not required.

A composition range within the above broad limits that has been found to be particularly adaptable for making commercial alloys comprises alloys containing chromium in amount between 18% to 22% by weight, carbon 0.8% to 1.25%, silicon in amount between 0.1% to 2%, molybdenum in amount between 0.5% to 3%, tungsten in amount between 0.5% to 3%, columbium in amount between 0.5% to 2%, nickel in amount between 2% to 6%, manganese in amount up to 7%, nitrogen in amount up to 0.3% with the balance essentially iron (Fe) and any incidental impurities. Alloys within these commercial ranges are machinable and readily welded and have remarkably high strengths and stability at high temperature up to 1800° F.

In evaluating heat resisting alloys for such application as gas turbine engines and the like, long time rupture tests at high temperatures and short-time tensile tests at room temperature and at elevated temperatures are desirable indicators of their effectiveness. Such tests have been made of the novel alloys of this invention using precision cast test bars, produced by the well known "lost wax" process, measuring about 0.25 inch in diameter and having a one-inch gauge length. For determining the suitability of the alloy for high temperature application, a long time test, so-called "stress rupture" test was used. In this test each of several specimens of the alloy was subjected to measured tensile stress at a particular elevated temperature, and the time required for the sample to fail under these conditions of temperature and stress was noted. Data obtained in this manner permits determination of a

100-hour or 1,000-hour rupture life of the alloy, which is the stress which will produce rupture in 100 hours or 1,000 hours, respectively at the temperature of test.

Another test which was employed in connection with the alloys of this invention is the so-called "tensile test" for evaluating the physical properties of the alloys. Short time tensile testing at high temperature is carried out in a standard tensile test machine equipped with a heated muffle for heating and maintaining the sample at temperature throughout the test. After one hour at temperature a tensile stress is gradually applied until the sample fails. After each test the sample is removed from the testing machine and allowed to cool to room temperature. The percentage elongation (percent El.), and the percent reduction area (percent A) are measured on each sample tested after cooling. The ultimate tensile strength (TS) is calculated as the maximum stress applied on the sample during testing.

A cast alloy is believed adequate when it has greater than 1% and preferably at least 2% elongation with at least 85,000 p.s.i. tensile at room temperature, a hot ten-

sile strength of at least 40,000 p.s.i. at 1500° F., with less than 35% elongation, and a 100-hour rupture life at a temperature of 1500° F., when subjected to a rupture stress of about 20,000 p.s.i. or higher.

The alloys produced in accordance with our invention have adequate strength and ductility at both room and elevated temperature; furthermore, they have a 100-hour rupture life at 1500° F., when subjected to a rupture stress of 20,000 p.s.i. and may attain as high as 28,000 p.s.i. in as cast condition and as high as 30,000 p.s.i. in the heat treated conditions.

In order to facilitate a better understanding of the invention and appreciation of its advantages, reference is made to Tables I and II below setting forth respectively, the composition of many alloys made in accordance with our invention and the short time tensile test and stress rupture test results obtained with such alloys in the manner described above. It will be understood that the examples given are by way of exemplification only and are not to be considered as limiting the scope of our invention thereto.

TABLE NO. 1  
Constituents of Alloys Tested

[Amounts given are in percent by weight]

| Alloy | C    | Cr    | Si   | W    | Mo   | Cb   | Ni   | Mn  | N | B                | P | Fe   |
|-------|------|-------|------|------|------|------|------|-----|---|------------------|---|------|
| 1     | 0.55 | 20    | 1    | 1.8  | 2    | 1    | 5    | 5   |   |                  |   | Bal. |
| 2     | 0.79 | 20    | 1    | 1.8  | 2    | 2    | 5    | 5   |   |                  |   | Bal. |
| 3     | 1.01 | 20    | 0.6  | 2    | 2    | 2    | 5    | 5   |   |                  |   | Bal. |
| 3A    | 0.96 | 20    | 0.6  | 2    | 2    | 2    | 5    | 5   |   |                  |   | Bal. |
| 3B    | 1.04 | 20    | 0.6  | 2    | 2    | 2    | 5    | 5   |   |                  |   | Bal. |
| 3C    | 1.03 | 20    | 0.6  | 2    | 2    | 2    | 5    | 5   |   |                  |   | Bal. |
| 3D    | 0.99 | 20    | 0.6  | 2    | 2    | 2    | 5    | 5   |   |                  |   | Bal. |
| 4     | 0.98 | 20    | 0.7  | 3    | 3    | 3    | 5    | 5   |   |                  |   | Bal. |
| 5     | 1.02 | 20    | 0.6  | 2    | 2    | 2    | 5    | 5   |   |                  |   | Bal. |
| 6     | 1.05 | 20.05 | 1.15 | 1.09 | 1.14 | 1.07 | 4.98 | 4.5 |   | 0.1              |   | 0.1  |
| 7     | 1.0  | 20    | 0.6  | 4    | 4    | 4    | 5    | 5   |   |                  |   | Bal. |
| 8     | 1    | 20    | 0.6  | 2    | 2    | 2    | 5    | 5   |   |                  |   | 0.2  |
| 9     | 0.98 | 20    | 0.6  | 2    | 2    | 2    | 5    | 5   |   |                  |   | Bal. |
| 10    | 1.08 | 20    | 1    | 2    | 2    | 2    | 5    | 5   |   |                  |   | 0.05 |
| 11    | 1.01 | 20    | 0.5  | 2    | 2    | 2    | 5    | 5   |   |                  |   | Bal. |
| 12    | 1.10 | 20    | 0.5  | 2    | 2    | 2    | 5    | 5   |   |                  |   | Bal. |
| 13    | 1.12 | 19.47 | 0.5  | 1.49 | 2.03 | 2.19 | 4.93 | 4.6 |   |                  |   | Bal. |
| 14    | 1.08 | 20    | 0.5  | 2    | 2    | 2    | 5    | 5   |   |                  |   | Bal. |
| 15    | 1.01 | 20.5  | 0.52 | 1.84 | 2.08 | 2.34 | 4.97 | 4.8 |   | 0.2 <sup>3</sup> |   | Bal. |
| 16    | 0.98 | 15    | 0.5  | 2    | 2    | 2    | 5    | 5   |   |                  |   | 0.1  |
| 17    | 1.16 | 25    | 0.5  | 2    | 2    | 2    | 5    | 5   |   |                  |   | Bal. |
| 18    | 0.97 | 20    | 0.5  | 2    | 2    | 2    | 4    | 7   |   |                  |   | 0.1  |
| 19    | 1.0  | 20    | 0.5  | 2    | 2    | 2    | 4    | 7   |   |                  |   | Bal. |
| 20    | 1.02 | 20    | 0.3  | 2    | 2    | 2    | 5    | 5   |   |                  |   | 0.1  |
| 21    | 0.96 | 20    | 0.5  | 2    | 4    | 2    | 5    | 5   |   |                  |   | Bal. |
| 22    | 0.93 | 20    | 0.5  | 2    | 7    | 2    | 5    | 5   |   |                  |   | Bal. |
| 23    | 1.0  | 20    | 1.0  | 2    | 2    | 2    | 5    | 5   |   |                  |   | Bal. |
| 24    | 1.03 | 20    | 1.5  | 2    | 2    | 2    | 5    | 5   |   |                  |   | Bal. |
| 25    | 1.07 | 20    | 2.0  | 2    | 2    | 2    | 5    | 5   |   |                  |   | Bal. |
| 26    | 1.04 | 20    | 0.5  | 2    | 2    | 2    | 4    | 7   |   |                  |   | Bal. |
| 27    | 1.05 | 20    | 0.5  | 1    | 2    | 2    | 5    | 5   |   |                  |   | Bal. |
| 28    | 0.97 | 20    | 0.5  | 2    | 2    | 1    | 5    | 5   |   |                  |   | Bal. |
| 29    | 0.90 | 20    | 0.5  | 1    | 2    | 1    | 5    | 5   |   |                  |   | 0.1  |
| 30    | 1.0  | 20    | 0.5  | 1    | 4    | 1    | 5    | 5   |   |                  |   | Bal. |
| 31    | 1.02 | 20    | 0.5  | 1    | 10   | 1    | 5    | 5   |   |                  |   | 0.1  |
| 32    | 1.02 | 20    | 0.5  | 1    | 2    | 2    | 5    | 5   |   |                  |   | 0.1  |
| 33    | 1.09 | 20    | 0.5  | 2    | 2    | 1    | 5    | 5   |   |                  |   | 0.1  |
| 34    | 0.93 | 20    | 0.5  | 1    | 2    | 2    | 5    | 5   |   |                  |   | Bal. |
| 35    | 0.81 | 20    | 0.5  | 1    | 2    | 4    | 5    | 5   |   |                  |   | Bal. |
| 36    | 0.98 | 20    | 0.5  | 1    | 10   | 1    | 5    | 5   |   |                  |   | 0.1  |
| 37    | 0.98 | 20    | 0.5  | 2    | 4    | 2    | 5    | 5   |   |                  |   | Bal. |
| 38    | 0.97 | 20    | 0.5  | 2    | 4    | 2    | 5    | 5   |   |                  |   | Bal. |
| 39    | 1.0  | 15    | 0.5  | 2    | 4    | 2    | 5    | 5   |   |                  |   | Bal. |
| 40    | 1.0  | 12    | 0.5  | 2    | 4    | 2    | 5    | 5   |   |                  |   | Bal. |
| 41    | 1.06 | 25    | 0.5  | 2    | 4    | 2    | 5    | 5   |   |                  |   | Bal. |
| 42    | 0.98 | 20    | 0.5  | 2    | 4    | 1.5  | 5    | 5   |   |                  |   | Bal. |
| 43    | 0.99 | 20    | 0.5  | 2    | 4    | 1.5  | 5    | 5   |   |                  |   | Bal. |
| 44    | 1.01 | 20    | 0.5  | 4    | 4    | 1    | 5    | 5   |   |                  |   | Bal. |
| 45    | 0.96 | 20    | 0.5  | 4    | 4    | 1    | 5    | 5   |   |                  |   | Bal. |
| 46    | 0.98 | 20    | 0.5  | 4    | 2    | 2    | 5    | 5   |   |                  |   | Bal. |
| 47    | 0.99 | 20    | 0.5  | 7    | 2    | 2    | 5    | 5   |   |                  |   | Bal. |
| 48    | 0.90 | 20    | 0.5  | 2    | 7    | 2    | 5    | 5   |   |                  |   | Bal. |
| 49    | 0.92 | 20    | 1.0  | 2    | 7    | 2    | 5    | 5   |   |                  |   | Bal. |
| 50    | 0.94 | 20    | 0.6  | 2    | 4    | 1    | 5    | 5   |   |                  |   | Bal. |
| 51    | 0.97 | 20    | 0.6  | 2    | 4    | 1    | 5    | 5   |   |                  |   | Bal. |
| 52    | 1.0  | 20    | 0.5  | 2    | 4    | 1    | 5    | 5   |   |                  |   | Bal. |
| 53    | 1.04 | 20    | 0.5  | 2    | 4    | 1    | 5    | 5   |   |                  |   | Bal. |
| 54    | 1.0  | 20    | 0.5  | 2    | 4    | 1    | 5    | 5   |   |                  |   | Bal. |
| 55    | 0.96 | 20    | 0.5  | 2    | 4    | 1    | 5    | 5   |   |                  |   | Bal. |
| 56    | 1.06 | 20    | 0.5  | 4    | 1    | 2    | 5    | 5   |   |                  |   | Bal. |
| 57    | 1.06 | 20    | 0.5  | 4    | 1    | 2    | 5    | 5   |   |                  |   | Bal. |
| 58    | 0.87 | 20    | 0.5  | 4    | 1    | 1    | 5    | 5   |   |                  |   | Bal. |
| 59    | 1.0  | 20    | 0.5  | 1    | 4    | 1    | 5    | 5   |   |                  |   | Bal. |

See footnotes at end of table.

TABLE NO. 1—Continued

[Amounts given are in percent by weight]

| Alloy | C    | Cr   | Si   | W   | Mo  | Cb  | Ni  | Mn  | N     | B     | P    | Fe                                         |
|-------|------|------|------|-----|-----|-----|-----|-----|-------|-------|------|--------------------------------------------|
| 60    | 1.03 | 20   | 0.5  | 3   | 4   | 1   | 5   | 5   | 0.3   | 0.1   | 0.1  | Bal.                                       |
| 61    | 1.03 | 20   | 0.5  | 3   | 3   | 1   | 5   | 5   | 0.3   | 0.1   | 0.1  | Bal.                                       |
| 62    | 1.24 | 20   | 0.5  | 4   | 4   | 1   | 5   | 5   | 0.3   | 0.1   | 0.1  | Bal.                                       |
| 63    | 1.04 | 20   | 0.5  | 3   | 3   | 1   | 5   | 5   | 0.3   | 0.1   | 0.1  | Bal.                                       |
| 64    | 1.03 | 20   | 0.5  | 2   | 2   | 2   | 5   | 5   | 0.3   | 0.1   | 0.1  | Bal. <sup>10</sup>                         |
| 65    | 1.07 | 20   | 0.5  | 2   | 2   | 1.5 | 5   | 5   | 0.3   | 0.1   | 0.1  | Bal.                                       |
| 66    | 1.64 | 20   | 0.5  | 4   | 4   | 1   | 5   | 5   | 0.3   | 0.1   | 0.1  | Bal.                                       |
| 67    | 1.38 | 20   | 0.5  | 2   | 2   | 2   | 4   | 7   | 0.5   | 0.1   | 0.1  | Bal.                                       |
| 68    | 0.98 | 20   | 0.5  | 2   | 2   | 2   | 2   | 10  | 0.5   | 0.1   | 0.1  | Bal.                                       |
| 69    | 1.74 | 20   | 0.5  | 4   | 4   | 1   | 5   | 5   | 0.3   | 0.1   | 0.1  | Bal.                                       |
| 70    | 1.02 | 20   | 0.5  | 2   | 2   | 2   | 5   | 5   | 0.025 | 0.1   | 0.1  | Bal.                                       |
| 71    | 1.09 | 20   | 0.5  | 2   | 2   | 2   | 5   | 5   | 0.15  | 0.1   | 0.1  | Bal.                                       |
| 72    | 1.10 | 20   | 0.5  | 2   | 2   | 2   | 5   | 5   | 0.2   | 0.1   | 0.1  | Bal.                                       |
| 73    | 1.07 | 20   | 0.5  | 2   | 2   | 2   | 2   | 15  | 0.9   | 0.1   | 0.1  | Bal.                                       |
| 74    | 1.10 | 20   | 0.5  | 2   | 2   | 2   | 2   | 10  | 0.5   | 0.1   | 0.1  | Bal.                                       |
| 75    | 1.04 | 20   | 0.5  | 2   | 2   | 2   | 5   | 5   | 0.3   | 0.1   | 0.1  | Bal.                                       |
| 76    | 0.82 | 20   | 0.5  | 2   | 2   | 2   | 5   | 5   | 0.3   | 0.1   | 0.1  | Bal.                                       |
| 77    | 0.62 | 20   | 0.5  | 2   | 2   | 2   | 2   | 8   | 0.3   | 0.1   | 0.1  | Bal.                                       |
| 78    | 1.09 | 20   | 0.5  | 2   | 2   | 2   | 2   | 4   | 10    | 0.5   | 0.1  | Bal.                                       |
| 79    | 1.04 | 20   | 0.5  | 2   | 2   | 2   | 2   | 7   | 10    | 0.5   | 0.1  | Bal.                                       |
| 80    | 1.09 | 20   | 0.5  | 2   | 2   | 2   | 2   | 6   | 0.3   | 0.1   | 0.1  | Bal.                                       |
| 81    | 1.02 | 20   | 0.5  | 2   | 2   | 2   | 2   | 5   | 0.3   | 0.1   | 0.1  | Bal.                                       |
| 82    | 0.81 | 20   | 0.5  | 2   | 2   | 2   | 2   | 4   | 0.3   | 0.1   | 0.1  | Bal.                                       |
| 83    | 1.06 | 20   | 0.5  | 2   | 2   | 2   | 2   | 3   | 0.3   | 0.1   | 0.1  | Bal.                                       |
| 84    | 1.01 | 20   | 0.5  | 2   | 2   | 2   | 2   | 2   | 0.3   | 0.1   | 0.1  | Bal.                                       |
| 85    | 1.02 | 20   | 0.5  | 2   | 2   | 2   | 2   | 2   | 0.3   | 0.1   | 0.1  | Bal.                                       |
| 86    | 1.05 | 20   | 0.5  | 2   | 2   | 2   | 2   | 5   | 5     | 0.075 | 0.1  | Bal.                                       |
| 87    | 1.04 | 20   | 0.5  | 2   | 2   | 2   | 2   | 5   | 5     | 0.075 | 0.1  | Bal.                                       |
| 88    | 1.02 | 20   | 0.5  | 2   | 2   | 2   | 2   | 5   | 5     | 0.15  | 0.1  | Bal.                                       |
| 89    | 1.0  | 20   | 0.5  | 1   | 1   | 1   | 1   | 5   | 5     | 0.1   | 0.1  | Bal.                                       |
| 90    | 1.0  | 20   | 0.5  | 1   | 1   | 1   | 1   | 5   | 5     | 0.1   | 0.1  | Bal.                                       |
| 91    | 0.56 | 20   | 0.5  | 2   | 1   | 1   | 1   | 5   | 5     | 0.3   | 0.1  | Bal.                                       |
| 92    | 0.89 | 20   | 0.5  | 1   | 1   | 1   | 1   | 5   | 5     | 0.1   | 0.1  | Bal.                                       |
| 93    | 0.91 | 20   | 0.5  | 0.5 | 0.5 | 0.5 | 0.5 | 5   | 5     | 0.1   | 0.1  | Bal.                                       |
| 94    | 0.92 | 20   | 0.5  | 0.5 | 1   | 1   | 1   | 5   | 5     | 0.1   | 0.1  | Bal.                                       |
| 95    | 1.02 | 20   | 0.5  | 1   | 1   | 2   | 2   | 2   | 0.5   | 0.1   | 0.1  | Bal.                                       |
| 96    | 0.96 | 22   | 0.5  | 2   | 1   | 1   | 1   | 4   | 0.5   | 0.1   | 0.1  | Bal.                                       |
| 97    | 0.98 | 20   | 0.5  | 2   | 2   | 2   | 2   | 2   | 0.5   | 0.1   | 0.1  | Bal.                                       |
| 98    | 0.98 | 20   | 0.5  | 2   | 2   | 2   | 2   | 2   | 0.3   | 0.1   | 0.1  | Bal.                                       |
| 99    | 0.95 | 15   | 0.5  | 2   | 2   | 2   | 2   | 2   | 0.3   | 0.1   | 0.1  | Bal.                                       |
| 100   | 0.99 | 25   | 0.5  | 2   | 2   | 2   | 2   | 2   | 0.5   | 0.1   | 0.1  | Bal.                                       |
| 101   | 0.88 | 20   | 0.5  | 2   | 2   | 2   | 2   | 2   | 0.05  | 0.1   | 0.1  | Bal.                                       |
| 102   | 0.99 | 20   | 0.5  | 1   | 1   | 1   | 1   | 5   | 5     | 0.1   | 0.1  | Bal. <sup>11</sup>                         |
| 103   | 0.99 | 20   | 0.5  | 1   | 1   | 1   | 1   | 5   | 5     | 0.1   | 0.1  | Bal.                                       |
| 104   | 1.18 | 20   | 0.5  | 1   | 2   | 2   | 2   | 5   | 5     | 0.4   | 0.1  | Bal.                                       |
| 105   | 1.20 | 20   | 0.5  | 2   | 2   | 2   | 2   | 5   | 5     | 0.1   | 0.1  | Bal.                                       |
| 106   | 0.99 | 20   | 0.5  | 2   | 2   | 2   | 2   | 5   | 5     | 0.1   | 0.1  | Bal.                                       |
| 107   | 1.04 | 20   | 0.5  | 1   | 1   | 1   | 1   | 35  | 0.42  | 0.12  | 0.26 | Bal.                                       |
| 108   | 0.72 | 28   | 0.5  | 1   | 1   | 1.6 | 1.6 | 7.3 | 7.6   | 0.12  | 0.26 | Bal.                                       |
| 109   | 0.72 | 22.8 | 0.45 | 1   | 1   | 1   | 1   | 5   | 5     | 0.1   | 0.1  | Bal.                                       |
| 110   | 1.03 | 25   | 0.5  | 1   | 3   | 1   | 1   | 5   | 5     | 0.1   | 0.1  | Bal.                                       |
| 111   | 1.03 | 20   | 0.5  | 2   | 3   | 1   | 1   | 35  | 2     | 0.25  | 0.25 | Bal.                                       |
| 112   | 1.03 | 29.5 | 0.3  | 8.8 | 8.8 | 2   | 2   | 5   | 5     | 0.1   | 0.1  | Bal. <sup>12</sup>                         |
| 113   | 1.05 | 20   | 0.5  | 2   | 2   | 2   | 2   | 5   | 5     | 0.1   | 0.1  | Bal.                                       |
| 114   | 1.00 | 20   | 0.5  | 1   | 1   | 1.5 | 0.5 | 5   | 5     | 0.1   | 0.1  | Bal.                                       |
| 115   | 1.06 | 20   | 1.0  | 1.8 | 2.0 | 1   | 1   | 5   | 5     | 0.7   | 0.3  | Bal.                                       |
| 116   | 1.01 | 20   | 0.5  | 2   | 2   | 2   | 2   | 4   | 5     | 0.3   | 0.3  | Bal.                                       |
| 117   | 1.17 | 20   | 0.5  | 2   | 2   | 2   | 2   | 5   | 5     | 0.3   | 0.3  | Bal.                                       |
| 118   | 1.01 | 20   | 0.5  | 2   | 2   | 2   | 2   | 1   | 5     | 0.3   | 0.3  | Bal.                                       |
| 119   | 1.41 | 20   | 0.5  | 1   | 1   | 1   | 1   | 5   | 5     | 0.3   | 0.3  | Bal.                                       |
| 120   | 0.83 | 20   | 0.5  | 1   | 1   | 1   | 1   | 5   | 5     | 0.1   | 0.1  | Bal.                                       |
| 121   | 0.98 | 20   | 0.5  | 2   | 2   | 2   | 2   | 5   | 5     | 0.1   | 0.1  | Bal.                                       |
| 122   | 1.04 | 20   | 0.5  | 1   | 1   | 1   | 1   | 5   | 5     | 0.1   | 0.1  | Bal.                                       |
| 123   | 0.54 | 20   | 0.5  | 1   | 1   | 1   | 1   | 5   | 5     | 0.1   | 0.1  | Bal.                                       |
| 124   | 0.38 | 20   | 0.5  | 1   | 1   | 1   | 1   | 5   | 5     | 0.1   | 0.1  | Bal.                                       |
| 125   | 1.04 | 20   | 3.0  | 2   | 2   | 2   | 2   | 5   | 5     | 0.3   | 0.3  | Bal.                                       |
| 126   | 0.96 | 20   | 0.5  | 4   | 4   | 4   | 4   | 5   | 5     | 0.3   | 0.3  | Bal.                                       |
| 127   | 1.03 | 20   | 0.5  | 4   | 4   | 4   | 4   | 5   | 5     | 0.3   | 0.3  | Bal.                                       |
| 128   | 1.07 | 20   | 0.5  | 0.2 | 0.2 | 0.2 | 0.2 | 5   | 5     | 0.1   | 0.1  | Bal.                                       |
| 129   | 1.00 | 20   | 0.5  | 0.8 | 0.8 | 0.8 | 0.8 | 5   | 5     | 0.1   | 0.1  | Bal.                                       |
| 130   | 1.02 | 20   | 0.5  | 1.5 | 1.5 | 1.5 | 1.5 | 5   | 5     | 0.1   | 0.1  | Bal.                                       |
| 131   | 1.01 | 20   | 0.5  | 1.0 | 1.0 | 1.0 | 1.0 | 5   | 2     | 0.1   | 0.1  | Bal.                                       |
| 132   | 1.00 | 20   | 0.5  | 1.0 | 1.0 | 1.0 | 1.0 | 5   | 5     | 0.1   | 0.1  | Bal.                                       |
| 133   | 1.02 | 20   | 0.5  | 1.0 | 1.0 | 1.0 | 1.0 | 18  | 1.19  | 1.26  | 1.0  | Bal.                                       |
| 134   | 0.34 | 18   | 5    | 5   | 5   | 5   | 5   | 18  | 1.19  | 1.26  | 1.0  | Bal.                                       |
| 135   | 0.26 | 18   | 5    | 5   | 5   | 5   | 5   | 5   | 5     | 1.26  | 1.0  | Bal.                                       |
| 136   | 1.02 | 20   | 0.5  | 1.0 | 1.0 | 1.0 | 1.0 | 5   | 5     | 0.3   | 0.3  | Bal.                                       |
| 86a   | 1.05 | 20   | 0.5  | 2.0 | 2.0 | 2.0 | 2.0 | 5   | 5     | 0.3   | 0.3  | Bal.                                       |
| 86b   | 1.05 | 20   | 0.5  | 2.0 | 2.0 | 2.0 | 2.0 | 10  | 0.3   | 0.3   | 0.5  | Bal.                                       |
| 86c   | 1.05 | 20   | 0.5  | 2.0 | 2.0 | 2.0 | 2.0 | 5   | 5     | 0.5   | 0.5  | Bal.                                       |
| 86d   | 1.05 | 20   | 0.5  | 2.0 | 2.0 | 2.0 | 2.0 | 5   | 5     | 0.5   | 0.5  | Bal. <sup>13</sup>                         |
| 267   | 1.12 | 18   | 0.5  | 1.0 | 1.0 | 1.0 | 1.0 | 5   | 5     | 0.1   | 0.1  | Bal. <sup>13</sup>                         |
| 302   | 1.04 | 18   | 0.5  | 1.0 | 1.0 | 1.0 | 1.0 | 5   | 5     | 0.1   | 0.1  | Bal. <sup>13</sup>                         |
| 303   | 0.99 | 20   | 0.5  | 0.1 | 0.1 | 0.1 | 0.1 | 5   | 5     | 0.1   | 0.1  | Bal. <sup>13</sup>                         |
| 304   | 1.01 | 20   | 0.5  | 2.0 | 2.0 | 2.0 | 2.0 | 2   | 2     | 0.1   | 0.1  | Made from elemental high purity materials. |

<sup>1</sup> Actual analysis.<sup>2</sup> Was 0.1 nominal.<sup>3</sup> Was 0.3 nominal.<sup>4</sup> Includes 1.0% tantalum.<sup>5</sup> Includes 2.0% tantalum.<sup>6</sup> Includes 1.0 Ti.<sup>7</sup> Includes 2.0 Ti.<sup>8</sup> Includes 1.0 V.<sup>9</sup> Includes 2.0 V.<sup>10</sup> Includes 0.5 Ti.<sup>11</sup> Includes 0.1 misch metal (essentially equal parts of rare earth metals such as Ce, La).<sup>12</sup> Includes 5.0 Co.<sup>13</sup> Made from elemental high purity materials.

15  
TABLE NO. II  
Test Data

| Alloy  | Short-Time Tensile Testing |             |             |             | Stress-Rupture Testing at 1,500° F. |            |             |                       | 5       | Alloy   | Short-Time Tensile Testing |             |             |             | Stress-Rupture Testing at 1,500° F. |            |             |                       |        |  |
|--------|----------------------------|-------------|-------------|-------------|-------------------------------------|------------|-------------|-----------------------|---------|---------|----------------------------|-------------|-------------|-------------|-------------------------------------|------------|-------------|-----------------------|--------|--|
|        | Room Temperature           |             | 1,500° F.   |             | Stress (p.s.i.)                     | Time, Hour | Percent El. | 100 Hr. Life (p.s.i.) |         |         | Room Temperature           |             | 1,500° F.   |             | Stress (p.s.i.)                     | Time, Hour | Percent El. | 100 Hr. Life (p.s.i.) |        |  |
|        | TS (p.s.i.)                | Percent El. | TS (p.s.i.) | Percent El. |                                     |            |             |                       |         |         | TS (p.s.i.)                | Percent El. | TS (p.s.i.) | Percent El. |                                     |            |             |                       |        |  |
| 1..... | 95,000                     | 5           | 31,800      | 24          | 15,000                              | 131        | 22          | 15,500                | 20      | 105,250 | 1.6                        | 45,850      | 18          | 22,500      | 275                                 | 10         | 25,000      |                       |        |  |
|        | 99,000                     | 6           | 36,500      | 35          | 17,000                              | 41         | 29          | 15,500                | 20      | 85,000  | 1.5                        | 45,000      | 16          | 25,000      | 132                                 | 14         | 25,000      |                       |        |  |
| 2..... | 99,000                     | 3           | 38,200      | 22          | 20,000                              | 111.1      | 17.5        | 22,500                | 7.5     | 20,000  | 15                         | 44,600      | 18          | 27,500      | 34                                  | 12         | 25,500      |                       |        |  |
| 3..... | 95,000                     | 5           | 40,000      | 22          | 22,500                              | 7.5        | 20          | 20,000                | 15      | 28..... | .....                      | 30,000      | 17          | 22,500      | 287                                 | 10         | 25,500      |                       |        |  |
| 3..... | 98,400                     | 3           | 47,000      | 20          | 20,000                              | 477        | 7.0         | 22,500                | 30      | 90,800  | 2                          | 50,600      | 17          | 22,500      | 144                                 | 18         | 25,500      |                       |        |  |
| 3A.... | 107,000                    | 4           | 50,200      | 15          | 20,000                              | 604        | 10.5        | 25,000                | 64      | 105,250 | 1.6                        | 49,100      | 17          | 25,000      | 41                                  | 18         | 25,500      |                       |        |  |
| 3B.... | 108,000                    | 2.5         | 50,750      | 15          | 20,000                              | 470        | 4.0         | 24,000                | 77      | 82,400  | 1                          | 50,500      | 20          | 20,000      | 110                                 | 17         | 20,000      |                       |        |  |
| 3C.... | 99,000                     | 1.5         | 52,500      | 13          | 20,000                              | 455        | 21          | 24,000                | 20      | 102,300 | 2.5                        | 43,200      | 15          | 22,500      | 245                                 | 9          | 25,000      |                       |        |  |
| 3D.... | 90,000                     | 1           | 55,000      | 10          | 20,000                              | 388        | 21          | 25,000                | 104     | 98,000  | 1                          | 43,800      | 15          | 25,000      | 128                                 | 9          | 25,000      |                       |        |  |
| 4..... | 104,000                    | 1           | 50,000      | 18          | 20,000                              | 189        | 20          | 21,000                | 25      | 104,450 | 2                          | 41,600      | 18          | 30,000      | 10.5                                | 50         | 25,500      |                       |        |  |
| 5..... | 105,000                    | 3           | 48,000      | 15          | 22,500                              | 53         | 20          | 25,000                | 15      | 106,250 | 2                          | 33,600      | 35          | 18,000      | 12                                  | 50         | 14,000      |                       |        |  |
| 5..... | 105,000                    | 3           | 48,000      | 15          | 22,500                              | 290        | 6           | 25,000                | 158     | 80,000  | 1                          | 31,150      | 38          | 17,500      | 20,000                              | 3.7        | 21,500      |                       |        |  |
| 5..... | 105,000                    | 3           | 48,000      | 15          | 25,000                              | 14         | .....       | 25,000                | 158     | 80,000  | 1                          | 72,250      | 1           | 22,500      | 7                                   | 21         | 21,500      |                       |        |  |
| 5..... | 105,000                    | 3           | 48,000      | 15          | 25,000                              | 45         | 14          | 25,000                | 132,500 | 119,250 | 1                          | 61,500      | 15          | 20,000      | 418                                 | 14         | 25,000      |                       |        |  |
| 5..... | 105,000                    | 3           | 48,000      | 15          | 25,000                              | 165        | 4.6         | 30,000                | 37      | 119,700 | 1                          | 60,500      | 13          | 22,500      | 130                                 | 16         | 24,000      |                       |        |  |
| 6..... | 105,000                    | 4           | 41,000      | 18          | 20,000                              | 1,215      | 7           | 27,000                | 30      | 119,700 | 1                          | 58,750      | 19          | 25,000      | 71.5                                | 20         | 25,000      |                       |        |  |
| 6..... | 105,000                    | 4           | 41,000      | 18          | 25,000                              | 306        | 7.5         | 25,000                | 125,0   | 114,100 | 1                          | 61,000      | 18          | 20,000      | 638                                 | 12         | 25,000      |                       |        |  |
| 7..... | 100,000                    | 1           | 45,000      | 8           | 20,000                              | 15         | 45          | 17,500                | 38      | 110,000 | 1                          | 60,300      | 17          | 22,500      | 130                                 | 16         | 24,000      |                       |        |  |
| 8..... | 95,000                     | 2           | 44,000      | 13          | 20,000                              | 193        | 6           | 22,500                | 55      | 123,000 | 1                          | 56,150      | 23          | 22,500      | 71.5                                | 20         | 20,000      |                       |        |  |
| 8..... | 93,500                     | 2           | 43,500      | 15          | 20,000                              | 37         | 11          | 22,500                | 37      | 125,000 | 1                          | 54,500      | 25          | 23,000      | 99                                  | 18         | 25,000      |                       |        |  |
| 9..... | 105,000                    | 2           | 43,800      | 19          | 20,000                              | 275        | 8           | 22,500                | 132,500 | 119,250 | 1                          | 49,000      | 23          | 27,500      | 44                                  | 17         | 25,000      |                       |        |  |
| 9..... | 100,100                    | 2.5         | 44,200      | 19          | 22,500                              | 81         | 10          | 22,000                | 20,5    | 122,000 | 1.5                        | 50,700      | 15          | 20,000      | 109                                 | 15         | 20,000      |                       |        |  |
| 10.... | 101,400                    | 2.5         | 42,750      | 16          | 25,000                              | 20.5       | 15          | 22,500                | 342     | 123,700 | 2                          | 49,600      | 15          | 22,500      | 51                                  | 18         | 20,000      |                       |        |  |
| 10.... | 111,100                    | 2.5         | 49,200      | 12          | 22,500                              | 342        | 3           | 25,000                | 312     | 122,000 | 1                          | 63,700      | 18          | 20,000      | 215                                 | 20         | 20,000      |                       |        |  |
| 10.... | 109,900                    | 2.5         | 48,175      | 17          | 22,000                              | 122        | 4           | 25,000                | 122,000 | 122,000 | 1                          | 62,150      | 10          | 22,500      | 70                                  | 20         | 21,500      |                       |        |  |
| 11.... | 109,000                    | 4           | 49,500      | 10          | 20,000                              | 1,282      | 9           | 25,000                | 122,000 | 107,000 | 1                          | 61,700      | 15          | 20,000      | 351.5                               | 19         | 23,000      |                       |        |  |
| 11.... | 114,800                    | 4           | 47,400      | 12          | 22,500                              | 765        | 5           | 24,000                | 40      | 123,000 | 1                          | 60,600      | 16          | 22,500      | 87.5                                | 27         | 20,000      |                       |        |  |
| 11.... | 105,600                    | 4           | 47,600      | 14          | 25,000                              | 159        | 5           | 25,000                | 159     | 60,500  | 1                          | 60,500      | 19          | 25,000      | 44                                  | 33         | 20,000      |                       |        |  |
| 12.... | 115,000                    | 4           | 47,000      | 15          | 22,500                              | 70         | 8           | 25,000                | 159     | 104,000 | 1                          | 63,500      | 24          | 22,500      | 155                                 | 27         | 20,000      |                       |        |  |
| 12.... | 123,250                    | 2           | 53,100      | 13          | 25,000                              | 274        | 10          | 27,500                | 94,600  | 94,600  | 1                          | 61,650      | 18          | 25,000      | 62                                  | 34         | 23,500      |                       |        |  |
| 13.... | 122,500                    | 5           | 52,800      | 14          | 25,000                              | 985.5      | 5           | 27,000                | 45      | 93,000  | 1                          | 63,400      | 4           | 25,000      | 28                                  | 12         | 23,000      |                       |        |  |
| 13.... | 117,100                    | 3           | 51,250      | 15          | 25,000                              | 445        | 7.5         | 27,000                | 45      | 93,000  | 1                          | 63,400      | 6           | 25,000      | 32.5                                | 37         | 23,000      |                       |        |  |
| 13.... | 121,300                    | 2           | 50,650      | 22          | 27,500                              | 131        | 8           | 25,000                | 36      | 130     | 44                         | 96,900      | 1           | 65,700      | 5                                   | 20,000     | 310.5       | 24                    | 20,000 |  |
| 14.... | 121,800                    | 3           | 54,200      | 11          | 25,000                              | 272        | 10          | 25,000                | 35.2    | 45      | 90,600                     | 1           | 64,250      | 14          | 22,500                              | 199        | 23          | 24,000                |        |  |
| 14.... | 119,600                    | 2           | 55,400      | 14          | 27,500                              | 84.5       | 12          | 27,000                | 46      | 104,400 | 3                          | 64,300      | 15          | 25,000      | 64                                  | 27         | 24,000      |                       |        |  |
| 15.... | 128,000                    | 3           | 52,900      | 16          | 30,000                              | 38         | 16          | 25,000                | 275     | 103,500 | 3                          | 56,500      | 16          | 22,500      | 131                                 | 15         | 23,000      |                       |        |  |
| 15.... | 122,000                    | 2           | 60,475      | 17          | 25,000                              | 111        | 12          | 27,000                | 50      | 100,500 | 3                          | 56,100      | 20          | 27,500      | 27                                  | 25         | 23,000      |                       |        |  |
| 16.... | 115,500                    | 3           | 50,900      | 18          | 30,000                              | 37.1       | 16          | 25,000                | 202     | 47      | 80,000                     | 3           | 68,000      | 5           | 22,500                              | 42         | 31          | 20,000                |        |  |
| 16.... | 113,250                    | 3           | 47,875      | 13          | 25,000                              | 395        | 4           | 25,000                | 7       | 88,500  | 2                          | 65,000      | 4           | 23,000      | 34                                  | 17         | 20,000      |                       |        |  |
| 17.... | 118,600                    | 2           | 46,500      | 13          | 30,000                              | 24.5       | 11          | 25,000                | 48      | 116,000 | 1                          | 61,300      | 5           | 30,000      | 18.5                                | 17         | 24,500      |                       |        |  |
| 17.... | 114,000                    | 2           | 39,625      | 40          | 22,500                              | 57         | 50          | 25,000                | 13,500  | 126,000 | 1                          | 59,000      | 17          | 22,500      | 198                                 | 18         | 24,500      |                       |        |  |
| 18.... | 96,400                     | 2           | 47,600      | 13          | 22,500                              | 146        | 8.5         | 25,000                | 76      | 13,500  | 1                          | 61,000      | 13          | 25,000      | 74                                  | 24         | 24,500      |                       |        |  |
| 18.... | 87,250                     | 2           | 45,500      | 14          | 25,000                              | 47         | 12          | 24,000                | 49      | 103,200 | 1                          | 56,500      | 16          | 22,500      | 90                                  | 22         | 24,500      |                       |        |  |
| 19.... | 123,000                    | 2           | 56,250      | 14          | 22,500                              | 159        | 8           | 25,000                | 50      | 104,650 | 1                          | 56,450      | 18          | 20,000      | 241                                 | 12         | 24,500      |                       |        |  |
| 19.... | 120,400                    | 2           | 55,000      | 15          | 25,000                              | 98         | 11          | 24,000                | 51      | 112,600 | 1                          | 56,000      | 13          | 25,000      | 27                                  | 22         | 24,500      |                       |        |  |
| 20.... | 102,500                    | 2           | 47,025      | 15          | 25,000                              | 155.5      | 8.5         | 26,500                | 60      | 100,100 | 1.5                        | 60,700      | 9           | 20,000      | 82                                  | 17         | 22,000      |                       |        |  |
| 20.... | 106,100                    | 3           | 46,900      | 11          | 27,500                              | 94         | 4           | 26,500                | 60      | 101,600 | 2                          | 59,600      | 10          | 22,500      | 55                                  | 26         | 19,000      |                       |        |  |
| 21.... | 117,250                    | 2           | 52,600      | 15          | 22,500                              | 222        | 9.5         | 25,000                | 52      | 82,500  | 2                          | 55,800      | 2           | 20,000      | 370                                 | 8          | 20,000      |                       |        |  |
| 21.... | 113,250                    | 2           | 52,600      | 14          | 25,000                              | 96.5       | 9           | 24,500                | 53      | 81,750  | 2                          | 52,850      | 9           | 22,500      | 84.5                                | 10         | 22,000      |                       |        |  |
| 22.... | 119,250                    | 2           | 50,400      | 13          | 22,500                              | 24         | 14          | 25,000                | 54      | 103.5   | 1                          | 48,300      | 2           | 25,000      | 25                                  | 12         | 22,000      |                       |        |  |
| 22.... | 119,250                    | 2           | 49,100      | 32          | 25,000                              | 103.5      | 18          | 22,000                | 55      | 109,900 | 1                          | 54,400      | 19          | 22,500      | 49                                  | 17         | 22,000      |                       |        |  |
| 22.... | 48,400                     | 21          | 27,500      | 18.5        | 25,000                              | 27,500     | 27          | 25,000                | 65      | 126,000 | 1                          | 53,100      | 16          | 25,000      | 27.5                                | 25         | 19,000      |                       |        |  |
| 23.... | 118,500                    | 2           | 48,200      | 13          | 22,500                              | 286        | 5           | 25,000                | 54      | 122,000 | 1                          | 61,500      | 14          | 22,500      | 238                                 | 10         | 20,000      |                       |        |  |
| 23.... | 110,000                    | 3           | 45,500      | 15          | 25,000                              | 92         | 9           | 24,500                | 55      | 126,000 | 1                          | 60,500      | 14          | 25,000      | 99                                  | 17         | 25,000      |                       |        |  |
| 24.... | 117,000                    | 3           | 49,000      | 14          | 22,500                              | 225        | 6           | 25,000                | 55      | 122,000 | 1                          | 61,900      | 15          | 22,500      | 173                                 | 17         | 24,000      |                       |        |  |
| 24.... | 48,000                     | 13          | 25,000      | 53.5        | 7                                   | 24,500     | 55          | 122,000               | 1       | 62,750  | 12                         | 25,000      | 75          | 29          | 24,000                              | 25         | 24,000      |                       |        |  |
| 25.... | 114,100                    | 2           | 43,650      | 19          | 20,000                              | 335.5      | 4           | 25,000                | 56      | 124,700 | 3                          | 59,500      | 15          | 25,000      | 159                                 | 14         | 24,000      |                       |        |  |
| 25.... | 110,750                    | 2           | 43,400      | 17          | 22,500                              | 81         | 8           | 23,000                | 70      | 111,125 | 2                          | 57,600      | 18          | 25,000      | 155                                 | 8          | 25,000      |                       |        |  |
| 26.... | 128,500                    | 2           | 57,600      | 14          | 22,500                              | 307        | 11          | 25,000                | 58      | 103,000 | 1                          | 61,200      | 9           | 22,500      | 205                                 | 15         | 24,000      |                       |        |  |
| 26.... | 121,600                    | 2           | 57,000      | 17          | 25,000                              | 98.5       | 15          | 25,000                | 59      | 124,000 | 3                          | 60,250      | 10          | 22,500      | 86.5                                | 18         | 24,000      |                       |        |  |
| 26.... | 54,250                     | 21          | 27,500      | 46          | 17.5                                | 25,000     | 57          | 111,125               |         |         |                            |             |             |             |                                     |            |             |                       |        |  |

TABLE NO. II—Continued

| Alloy | Short-Time Tensile Testing |             |             |             | Stress-Rupture Testing at 1,500° F. |            |             |                       | 5   | Short-Time Tensile Testing |             |             |             | Stress-Rupture Testing at 1,500° F. |            |             |                       |         |
|-------|----------------------------|-------------|-------------|-------------|-------------------------------------|------------|-------------|-----------------------|-----|----------------------------|-------------|-------------|-------------|-------------------------------------|------------|-------------|-----------------------|---------|
|       | Room Temperature           |             | 1,500° F.   |             | Stress (p.s.i.)                     | Time, Hour | Percent El. | 100 Hr. Life (p.s.i.) |     | Room Temperature           |             | 1,500° F.   |             | Stress (p.s.i.)                     | Time, Hour | Percent El. | 100 Hr. Life (p.s.i.) |         |
|       | TS (p.s.i.)                | Percent El. | TS (p.s.i.) | Percent El. |                                     |            |             |                       |     | TS (p.s.i.)                | Percent El. | TS (p.s.i.) | Percent El. |                                     |            |             |                       |         |
| 60    | 116,000                    | 3           | 62,000      | 18          | 22,500                              | 156.5      | 22          | 24,000                | 92  | 117,200                    | 2.5         | 59,800      | 13          | 22,500                              | 311.5      | 10          |                       |         |
|       |                            |             | 62,000      | 22          | 27,500                              | 33         | 22          |                       |     |                            |             |             |             | 25,000                              | 79         | 14          | 25,000                |         |
| 61    | 100,775                    | 1           | 59,500      | 10          | 25,000                              | 76.5       | 23          |                       | 15  | 93                         | 111,000     | 1.5         | 52,800      | 14                                  | 22,500     | 212         | 8.5                   |         |
| 62    | 115,750                    | 1           | 62,000      | 11          | 30,000                              | 19         | 17          | 24,000                |     |                            |             |             |             | 25,000                              | 76         | 11          | 24,000                |         |
|       |                            |             | 68,000      | 10          | 30,000                              | 183        | 9           | 27,000                |     |                            |             |             |             | 27,000                              | 32.4       | 14          |                       |         |
| 63    | 118,000                    | 2           | 63,400      | 11          | 25,000                              | 101        | 21          |                       |     |                            |             |             |             | 102,800                             | 4          | 50,000      | 16                    | 22,500  |
|       |                            |             | 64,000      | 12          | 27,500                              | 44         | 20          | 25,000                | 95  |                            |             |             |             | 44,300                              | 17         | 25,000      | 101                   | 8       |
| 64    | 123,000                    | 2           | 60,000      | 16          | 22,500                              | 462        | 13          |                       | 20  |                            |             |             |             | 44,200                              | 17         | 27,500      | 19                    | 18      |
|       |                            |             | 59,000      | 19          | 25,000                              | 80         | 15          | 25,000                | 93  |                            |             |             |             | 106,400                             | 1.5        | 49,600      | 13                    | 25,000  |
| 65    | 90,000                     | 2.5         | 48,650      | 5           | 22,500                              | 187        | 7           |                       |     |                            |             |             |             | 123,000                             | 1.5        | 48,000      | 11                    | 15,000  |
|       |                            |             | 48,800      | 5           | 25,000                              | 65         | 6.5         | 23,500                |     |                            |             |             |             | 10,000                              | 6          | 43          |                       | 10,000  |
| 66    | Brittle                    |             | 44,550      | 10          | 27,500                              | 15         | 10          |                       |     |                            |             |             |             | 105,200                             | 1.5        | 21,000      | 33                    | 27,500  |
|       |                            |             | 76,000      | 2           | 25,000                              | 334        | 14.5        |                       |     |                            |             |             |             | 123,000                             | 3          | 53,000      | 15                    | 20,000  |
| 67    | 126,600                    | 1           | 66,500      | 9           | 27,500                              | 146.5      | 18          | 28,000                | 25  | 99                         | 113,300     | 3           | 42,700      | 14                                  | 23,000     | 29          | 0.2                   | 42      |
|       |                            |             | 63,000      | 13          | 25,000                              | 258        | 12          | 28,000                |     |                            |             |             |             | 113,300                             | 3          | 42,700      | 14                    | 6,000   |
| 68    | 123,600                    | 2.5         | 64,200      | 13          | 27,500                              | 389        | 2.5         |                       |     |                            |             |             |             | 85,000                              | 1          | 21,000      | 30                    | 19,000  |
|       |                            |             | 65,000      | 16          | 25,000                              | 127        | 15          | 28,000                |     |                            |             |             |             | 120,000                             | 2          | 41,750      | 14                    | 38.8    |
| 69    | 101,000                    | 1           | 73,000      | 3           | 25,000                              | 148.5      | 22.5        |                       | 30  |                            |             |             |             | 108,800                             | 2          | 48,250      | 12                    | 17,500  |
|       |                            |             | 69,500      | 6           | 27,500                              | 77         | 23          | 26,500                |     |                            |             |             |             | 108,800                             | 2          | 48,250      | 12                    | 162.5   |
| 70    | 100,500                    | 1           | 49,300      | 17          | 25,000                              | 155        | 5           |                       |     |                            |             |             |             | 119,500                             | 3          | 49,600      | 17                    | 25,000  |
| 71    | 106,100                    | 2           | 49,750      | 21          | 25,000                              | 313        | 4           |                       |     |                            |             |             |             | 102,200                             | 3          | 43,300      | 17                    | 30,000  |
| 72    | 98,000                     | 1           | 50,300      | 14          | 22,500                              | 195        | 3.5         |                       |     |                            |             |             |             | 105,000                             | 2.5        | 45,850      | 13                    | 25,000  |
|       |                            |             | 25,000      | 103         | 5                                   | 25,000     | 35          | 104                   |     |                            |             |             |             | 119,500                             | 3          | 49,600      | 17                    | 22,500  |
| 73    | 111,600                    | 2           | 53,100      | 14          | 22,500                              | 345        | 3.5         | 25,000                |     |                            |             |             |             | 105,000                             | 2.5        | 45,850      | 13                    | 22,500  |
|       |                            |             | 25,000      | 88          | 10                                  | 25,000     | 105         |                       |     |                            |             |             |             | 119,500                             | 3          | 49,600      | 17                    | 22,500  |
| 74    | 134,200                    | 1           | 59,600      | 14          | 20,000                              | 51.5       | 14          | 18,000                | 40  | 106                        | 118,000     | 1           | 53,150      | 15                                  | 27,500     | 98          | 16                    |         |
| 75    | 125,000                    | 1           | 60,000      | 7           | 25,000                              | 116.5      | 3.5         |                       |     |                            |             |             |             | 100,050                             | 3          | 44,000      | 20                    | 25,000  |
| 76    | 95,000                     | 1           | 48,900      | 11          | 22,500                              | 236.5      | 12          |                       |     |                            |             |             |             | 108                                 |            |             |                       | 27,500  |
|       |                            |             | 25,000      | 133         | 6                                   | 25,500     |             |                       |     |                            |             |             |             |                                     |            |             | 125,000               |         |
| 77    | 111,300                    | 4           | 50,300      | 13          | 20,000                              | 198.5      | 12          |                       | 45  |                            |             |             |             | 106,000                             | 2          | 54,500      | 16                    | 340,000 |
|       |                            |             | 22,500      | 66          | 21                                  | 22,000     |             |                       |     |                            |             |             |             | 106,000                             | 2          | 54,500      | 16                    | 45,000  |
| 78    | 115,000                    | 3           | 55,200      | 11          | 20,000                              | 278        | 3.5         |                       | 109 |                            |             |             |             | 106,000                             | 2          | 54,500      | 16                    | 40,000  |
|       |                            |             | 22,000      | 119.5       | 3                                   | 23,000     |             |                       |     |                            |             |             |             | 110                                 |            |             |                       | 45,000  |
| 79    | 100,100                    | 1           | 56,000      | 18          | 20,000                              | 168        | 10          |                       |     |                            |             |             |             | 101,000                             | 1          | 59,000      | 12                    | 25,000  |
|       |                            |             | 22,500      | 73          | 8                                   | 22,000     |             |                       |     |                            |             |             |             | 111                                 |            |             |                       | 25,000  |
| 80    | 73,100                     | 1           | 55,300      | 4           | 17,500                              | 151        | 1.5         |                       |     |                            |             |             |             | 112                                 |            | 77,500      | 1                     | 24,000  |
| 81    | 114,000                    | 3           | 57,000      | 10          | 22,500                              | 159.5      | 4           |                       |     |                            |             |             |             | 113                                 |            | 110,000     | 2                     | 52,300  |
|       |                            |             | 53,600      | 10          | 27,500                              | 36         | 5.5         |                       |     |                            |             |             |             | 113                                 |            | 110,000     | 2                     | 52,300  |
| 82    | 120,000                    | 2.5         | 54,700      | 12          | 20,000                              | 300        | 3.5         |                       |     |                            |             |             |             | 104,600                             | 2          | 51,200      | 14                    | 25,000  |
|       |                            |             | 52,400      | 15          | 22,500                              | 94         | 2.5         | 23,000                | 55  |                            |             |             |             | 114                                 |            | 104,600     | 2                     | 51,200  |
| 83    | 125,150                    | 3           | 57,000      | 12          | 20,000                              | 252        | 3           |                       |     |                            |             |             |             | 115                                 |            | 101,000     | ---                   | 57,000  |
|       |                            |             | 56,000      | 13          | 22,500                              | 88.5       | 3.5         | 23,000                |     |                            |             |             |             | 115                                 |            | 101,000     | ---                   | 57,000  |
| 84    | 122,800                    | 4           | 54,000      | 17          | 22,500                              | 152        | 7           | 24,000                | 60  | 116                        | 123,600     | 2           | 59,000      | 16                                  | 123,600    | 2           | 59,000                |         |
|       |                            |             | 25,000      | 89.5        | 7                                   | 24,000     |             |                       |     |                            |             |             |             | 116                                 |            | 123,600     | 2                     | 59,000  |
| 85    | 121,000                    | 4           | 50,450      | 15          | 22,500                              | 196        | 5           |                       |     |                            |             |             |             | 117                                 |            | 123,200     | 1.5                   | 65,000  |
|       |                            |             | 25,000      | 73.5        | 6                                   | 24,000     |             |                       |     |                            |             |             |             | 117                                 |            | 123,200     | 1.5                   | 65,000  |
| 86    | 112,000                    | 1.5         | 47,500      | 9           | 17,500                              | 17         | 52          | 6,000                 |     |                            |             |             |             | 118                                 |            | 114,000     | 2                     | 55,000  |
|       |                            |             | 25,000      | 0.1         | 32                                  |            |             |                       |     |                            |             |             |             | 118                                 |            | 114,000     | 2                     | 55,000  |
| 87    | 105,000                    | 1           | 48,000      | 21          | 22,500                              | 290        | 10          |                       |     |                            |             |             |             | 119                                 |            | 97,500      | 1                     | 53,500  |
|       |                            |             | 25,000      | 80          | 14                                  | 24,000     | 65          |                       |     |                            |             |             |             | 119                                 |            | 97,500      | 1                     | 53,500  |
| 88    | 112,100                    | 3           | 50,000      | 21          | 22,500                              | 42         | 14          |                       |     |                            |             |             |             | 120                                 |            | 102,000     | 2                     | 42,750  |
|       |                            |             | 25,000      | 25          | 10                                  |            |             |                       |     |                            |             |             |             | 120                                 |            | 102,000     | 2                     | 42,750  |
| 89    | 121,500                    | 3           | 51,000      | 21          | 22,500                              | 630        | 6           |                       |     |                            |             |             |             | 120                                 |            | 116,030     | 2.5                   | 54,000  |
|       |                            |             | 25,000      | 253         | 12                                  | 27,000     | 70          | 121                   |     |                            |             |             |             | 121                                 |            | 116,030     | 2.5                   | 54,000  |
| 90    | 109,100                    | 3           | 48,600      | 19          | 25,000                              | 104.5      | 17.5        |                       |     |                            |             |             |             | 120                                 |            | 104,000     | 6                     | 42,750  |
|       |                            |             | 25,000      | 45          | 15                                  | 25,500     |             |                       |     |                            |             |             |             | 120                                 |            | 104,000     | 6                     | 42,750  |
| 91    | 108,200                    | 4           | 45,750      | 24          | 27,500                              | 39         | 19          |                       |     |                            |             |             |             | 122                                 |            | 105,000     | 2                     | 47,100  |
|       |                            |             | 49,700      | 28          | 20,000                              | 44         | 25          | 18,250                | 123 |                            |             |             |             | 122                                 |            | 105,000     | 2                     | 47,100  |
|       |                            |             | 42,700      | 31          | 22,500                              | 21.5       | 35          |                       |     |                            |             |             |             | 123                                 |            | 113,000     | 12                    | 36,400  |
|       |                            |             | 25,000      | 6.5         | 32                                  |            |             |                       |     |                            |             |             |             | 123                                 |            | 113,000     | 12                    | 36,400  |
|       |                            |             |             |             |                                     |            |             |                       |     |                            |             |             |             | 75                                  |            |             |                       |         |

TABLE NO. II—Continued

TABLE NO. II—Continued

| Alloy  | Short-Time Tensile Testing |             |             |             | Stress-Rupture Testing at 1,500° F. |            |             |                       |
|--------|----------------------------|-------------|-------------|-------------|-------------------------------------|------------|-------------|-----------------------|
|        | Room Temperature           |             | 1,500° F.   |             | Stress (p.s.i.)                     | Time, Hour | Percent El. | 100 Hr. Life (p.s.i.) |
|        | TS (p.s.i.)                | Percent El. | TS (p.s.i.) | Percent El. |                                     |            |             |                       |
| 124... | 110,000                    | 14          | 30,600      | 46          | 17,500                              | 17.5       | 49          | 14,500                |
| 125... | 96,500                     | 1           | 40,000      | 30          | 15,000                              | 87.5       | 33          | 15,500                |
| 126... | 111,500                    | 2           | 56,700      | 11          | 20,000                              | 13         | 36          | 15,500                |
| 127... | 105,800                    | 3           | 56,000      | 14          | 25,000                              | 2.8        | 85          | 15,500                |
| 128... | 107,000                    | 1           | 48,000      | 15          | 17,500                              | 40.5       | 28          | 15,500                |
| 129... | 100,000                    | 4           | 42,600      | 25          | 25,000                              | 54         | 26          | 22,000                |
| 130... | 100,000                    | 3           | 45,000      | 17.5        | 22,500                              | 75.3       | 20          | 15,500                |
| 131... | 100,500                    | 3           | 44,500      | 17.5        | 25,000                              | 261        | 15.5        | 25,000                |
| 132... | 93,600                     | 2           | 45,300      | 18          | 27,000                              | 87.3       | 17          | 25,000                |
| 133... | 100,000                    | 3           | 42,000      | 13          | 22,500                              | 102.5      | 18          | 20,000                |
| 134... | 81,500                     | 1           | 59,000      | 5           | 25,000                              | 79.6       | 16          | 15,500                |
| 135... | 85,000                     | 1           | 55,000      | 8           | 22,500                              | 253        | 9           | 15,500                |
| 136... | 67,200                     | 1           | 62,000      | 1           | 25,000                              | 185        | 11          | 15,500                |
| 86a... | 133,000                    | 2           | 53,000      | 22          | 25,000                              | 74         | 7           | 15,500                |
| 86b... | 124,500                    | 2           | 54,000      | 20          | 22,500                              | 178        | 13          | 15,500                |
| 86c... | 123,000                    | 1           | 56,000      | 15.5        | 25,000                              | 121.5      | 15          | 15,500                |
| 86d... | 123,500                    | 1           | 62,000      | 12          | 22,500                              | 50.3       | 21          | 15,500                |
| 267... |                            |             |             |             | 27,500                              | 264        | 15          | 24,000                |
| 302... | 108,600                    | 3           |             |             | 27,500                              | 41         | 22          | 24,000                |
| 303... | 105,700                    | 6           | 41,500      | 21          | 25,000                              | 14.5       | 12          | 24,000                |
| 304... | 116,200                    | 2           |             |             | 22,500                              | 240        | 10.5        | 24,000                |
|        |                            |             |             |             | 27,500                              | 9.5        | 12          | 24,000                |
|        |                            |             |             |             | 22,500                              | 158        | 4           | 24,000                |
|        |                            |             |             |             | 25,000                              | 168        | 3.5         | 24,000                |
|        |                            |             |             |             | 27,500                              | 15         | 9           | 24,000                |
|        |                            |             |             |             | 25,000                              | 273        | 12          | 24,000                |
|        |                            |             |             |             | 27,500                              | 80.5       | 11          | 27,500                |
|        |                            |             |             |             | 30,000                              | 50         | 16          | 30,000                |
|        |                            |             |             |             | 22,500                              | 187        | 24          | 24,000                |
|        |                            |             |             |             | 25,000                              | 56         | 14          | 24,000                |
|        |                            |             |             |             | 27,500                              | 45.5       | 17          | 24,000                |
|        |                            |             |             |             | 25,000                              | 173        | 13          | 24,000                |
|        |                            |             |             |             | 27,500                              | 92         | 8           | 27,000                |
|        |                            |             |             |             | 22,500                              | 80.0       | 6           | 19,000                |
|        |                            |             |             |             | 22,500                              | 51.4       | 6           | 19,000                |
|        |                            |             |             |             | 25,000                              | 34.0       | 7           | 19,000                |
|        |                            |             |             |             | 22,500                              | 142.6      | 18          | 23,500                |
|        |                            |             |             |             | 25,000                              | 66.1       | 21          | 23,500                |
|        |                            |             |             |             | 27,500                              | 39.2       | 20          | 23,500                |
|        |                            |             |             |             | 22,500                              | 107        | 13          | 23,000                |
|        |                            |             |             |             | 25,000                              | 65.2       | 15          | 23,000                |
|        |                            |             |             |             | 27,500                              | 19.2       | 14          | 23,000                |
|        |                            |             |             |             | 22,500                              | 119        | 11          | 24,000                |
|        |                            |             |             |             | 25,000                              | 93.0       | 13          | 24,000                |
|        |                            |             |             |             | 27,500                              | 50.5       | 16          | 24,000                |
|        |                            |             |             |             | 22,500                              | 271.6      | 13          | 24,000                |
|        |                            |             |             |             | 25,000                              | 88.6       | 19          | 24,500                |
|        |                            |             |             |             | 27,000                              | 58.9       | 12          | 24,500                |
|        |                            |             |             |             | 25,000                              | 124        | 15          | 25,500                |
|        |                            |             |             |             | 27,000                              | 47.2       | 17          | 25,500                |
|        |                            |             |             |             | 30,000                              | 10.6       | 20          | 25,500                |
|        |                            |             |             |             | 20,000                              | 350.7      | 3           | 22,500                |
|        |                            |             |             |             | 22,500                              | 102.7      | 9           | 22,500                |
|        |                            |             |             |             | 25,000                              | 19.6       | 23          | 22,500                |
|        |                            |             |             |             | 18,000                              | 107        | 3           | 18,000                |
|        |                            |             |             |             | 22,500                              | 26.4       | 3           | 18,000                |
|        |                            |             |             |             | 25,000                              | 12.9       | 4           | 18,000                |

<sup>1</sup> Solution heat treated condition, 2,150° F./1 hr.+oil quench.<sup>2</sup> Stress rupture tested at 1,700° F.<sup>3</sup> Tested at 1,350° F.<sup>4</sup> Tested at 1,200° F.<sup>5</sup> Tested at 1,650° F.<sup>6</sup> Tested at 1,800° F.

In each example given in the tables the alloy was prepared either from relatively pure starting ingredients or from commercial grade source materials such as electrolytic grade iron for iron, ferro alloys of chromium, molybdenum, tungsten, and columbium for each of these metals, commercial grades of electrolytic nickel and electrolytic manganese for these substances and high carbon ferro-chrome as a source of carbon. In some instances the iron component was derived from SAE 1010 steel or Armco iron. Melting of proper proportions of the ingredients was normally carried out in a magnesia crucible and sometimes in a zircon or zirconia crucible and in each case in a high frequency induction furnace with the melt protected by an argon blanket or under a blanket of slag.

As previously noted that cast alloys may contain contaminating elements present by reason of using commercial alloy starting materials, by pickup from the crucible, etc. Although all of the alloys produced will possess physical properties within the limits given for a

5 alloy composition of the essential ingredients these contaminants may to some degree affect the 100 hour stress rupture values, such depending on the batch of commercial grade materials employed and the kind and number of contaminants contained therein. Such effects may be understood by a comparison for example of alloy Nos. 6 and 302, the former being made using relatively pure materials and the latter commercial grade ingredients. It is recommended that where the alloys are not prepared using relative pure starting materials that the complete chemical analysis be obtained of the starting ingredients for in this way the compositions may be controlled and deviations in properties explained.

Melts of the alloys recorded in the tables were cast in standard investment molds or ceramic shell molds produced by the "lost wax" process to obtain precision cast test bars. Each cast alloy was subjected to the stated short time tensile testing at room temperature and at 1500° F. and at a plurality of stress levels. The results of these tests recorded in Table II demonstrate the outstanding characteristics of the alloys of our invention.

The effect of varying the concentration of the essential ingredients of the alloys of our invention are evident from the many examples given in the tables. For the purpose of discussing some aspects thereof reference will be made to the effects obtained on a composition containing 20% Cr, 5% Ni, and 5% Mn. It will be understood that such is not to be construed as limiting such alloys to these specific values for other heats show the effects on other compositions.

Thus the effect of varying carbon additions on the properties of such a basic alloy is to be observed for example from the composition and test data for the following groups of heat numbers and from the graphs in FIGURE 8. Thus heats 124, 123, 120, 6, 104, and 119 show the effect of varying the carbon content using a 1% level of W, Mo and Cb and approximately 0.5 Si. Heats 1, 2, and 15 show the effect at levels of 2% each of W, and Mo and 1% Co and 0.5% to 1% Si. Heats 91, 13, and 105 show the effect of carbon at similar levels of W, Mo, Cb and Si where about 0.1 N is included. Heats 77, 76, 15, and 117 show the effect of carbon at levels of 2% each of W, Mo, and Cb, 0.5% Si and 0.3% N. Heats 45, 62, 66, and 69 show the effects of varying carbon at a 4% level of W and Mo, 1% of Cb, 0.5% Si, and 0.3 N.

50 This data reveals that the optimum high temperature properties are achieved at critical levels of carbon. For instance, lowering the carbon content substantially below about the 1% level for instance below 0.8% causes considerable weakening of the alloy whereas in general raising such amount substantially above the 1.25% level does not appreciably strengthen the same. It should also be noted that the optimum level of carbon increases with increasing concentrations of the NaCl-type of carbide forming elements. Moreover, those alloys containing amounts of carbon substantially above 1.25% exhibit low and inadequate cold ductility for many applications. Hence any potential improvement in strength due to higher carbon concentrations substantially above 1.25% appears to be without substantial practical value.

60 As described above, certain advantages result from the presence of nitrogen in the austenitic alloys of our invention. The effect of various concentrations up to 0.7% thereof is apparent, for example, from a consideration of the mechanical properties of an alloy composition containing 20% Cr, 5% Ni, 5% Mn, 1% C, and 0.5% silicon at different levels of W, Mo, and Cb as recorded for heat Nos. 3, 12, 13, 89, 14, 15, 106, 64 when 2% each of W, Mo and Cb were used. Heats 18, 26, 67, and 116 show the effect at the same level of the carbide formers but at 7% level of Mn and 4% Ni. Heats 6, 102, 90, and 92 show the effect at a 1% level of W, Mo, and Cb. Nitrogen is an effective austenite former and a potent strengthener through its formation of simple and complex nitrides. Significantly it improves the hot strength of the composi-

tion in the range 0.05% to 0.3% and without apparent loss in cold tensile ductility. Alloys 12-15 displayed outstanding creep strengths at 1500°, these registering stress rupture values of 27,000 p.s.i. after 100 hours. The best stress rupture value at 100 hours however with some sacrifice in the cold ductility properties was given by alloy 67 in which the nitrogen concentration was 0.5%. This alloy contained as noted, 4% Ni and 7 Mn. It had a strength of 28,000 p.s.i. Alloy 12 on the other hand containing 0.05% nitrogen and 5% each of Ni and Mn had a 100 hour rupture strength of 27,500 p.s.i. with good cold ductility. Somewhat lower ultimate creep rupture strengths were obtained using amounts of nitrogen in the same range when the W, Mo and Cb concentration was lowered from 2% to 1% as in alloys 6, 102, 90, and 92. In these instances however, the hot tensile strength was increased with increasing quantities of nitrogen. Alloy 195 containing 0.3% nitrogen, 5% manganese, and 2% of each of W, Mo, and Cb showed exceptionally good properties in the absence of both nickel and cobalt.

The effect of varying amounts of chromium in a basic composition containing for instance 5% Ni, 5% Mn, 1% C, and 0.5% Si were considered. The tables indicate that best results are to be expected from concentrations between about 12% to 20% of chromium at these levels of austenite formers. At 25% chromium the creep rupture strength dropped materially. Apparently this alloy becomes structurally unstable at this concentration. See and compare, for example, alloys 16, 10, and 17. Stable alloys using larger amounts of chromium than 20% can be obtained as evident from a consideration of heats 40, 39, 38, and 41 by employing greater amounts of austenite formers, in this instance nitrogen being used.

The effects of varying the total concentration of the carbide formers W, Mo, and Cb when used in multiple in the ratio of 1:1:1 will be seen from a comparison of the properties of alloys 129, 94, 6, 3, 4, 7, and 303 in connection with a composition containing 20 Cr, 5% Ni, 5% Mn, 1% C, and 0.5% Si.

In this illustration best properties were obtained at the 1% level of the carbide formers. When nitrogen in amounts of about 0.1% were added as in heats 93, 90, and 13 the best results were obtained at a higher level of the carbide formers W, Mo and Cb for instance 2% each. It will be observed that the best combination of properties is produced by a composition such as alloy No. 6 containing about 3% total, of the carbide forming elements W, Mo, and Cb in the ratio of 1:1:1. This alloy combines good cold tensile ductility (4% elongation) with an excellent 100 hour stress rupture value of 27,000 p.s.i. at 1500° F.

Varying the relative concentration of the individual strengtheners molybdenum, tungsten and columbium while still using them in multiple had different results. Alloys 6, 29, 30, 31 using a 1% level of each of W and Cb indicate some slight lowering in general of stress-rupture strengths at 100 hours for increasing amounts of Mo. Alloys 3, 21, and 22 show the effect of increasing amounts of Mo at the 2% level of each of W and Cb. Alloys 57, 56, 46, and 45 show the effect where unequal and greater amounts of W and Cb were used for instance 4% W, 2% Cb and 0.3% N was present. The same was true of tungsten with fixed equal and unequal amounts of Mo and Cb as demonstrated by alloys 15, 46, and 47 employing 2% each of Mo and Cb and alloys; 58, 59, 54, 60, and 45 containing 4% Mo and 1% Cb. Similar results were obtained by varying the columbium with fixed unequal concentrations of Mo and W as seen from alloys 29, 32, and 35.

In the case of the specific examples set forth where the 70 individual concentrations of Mo, W and Cb were quite high, 6% and more, there were marked drops in stress rupture strength apparent but increases in the hot tensile strength properties.

The addition of fourth and fifth NaCl carbide forming 75

strengthening elements, for example, titanium (Ti) and vanadium (V) on compositions of the invention is somewhat evident from alloys 43, 50, 52, 51, and 53. Thus increasing concentrations of titanium progressively lowered the hot strength properties and increased amounts of vanadium lowered the long time stress-rupture values and the hot strength at 1500° F. Such additions moreover produced alloys more difficult to cast. Moreover, mold reactions in preparation and excessive oxidation at 1500° F. were observed, such apparently accounting in some degree for their lower high temperature strengths.

Use of less than about 2% nickel in the absence of adequate manganese produces alloys having low stress-rupture strengths, due to structural instability of the austenite matrix. On the other hand, although substantial amounts of nickel up to about 20% may be used, additions of nickel substantially above the 2% to 8% level do not produce significant benefits. These results may be noted, for example, from the properties of alloys 86, 118, 85, 84, 83, 82, 81, and 78 at the level of 0.3% N with Mn omitted. Alloys 75, 79, 80 and 304 show the effects where amounts of Ni from 0% to 7% were used, alloys 75, 79 and 80 comprising alloys containing 10% Mn, 0.5% N, and 0.1% P and alloy 304 containing no manganese or nitrogen.

The effect of silicon (Si) upon the mechanical properties of a composition having 20% Cr, 5% Ni, 5% Mn, 2% Mo, 2% Cb, and 1% C is evident from alloys 3, 23, 24, 25, and 125. These results show that up to about 2% silicon does not adversely affect mechanical properties and a 3% level apparently causes embrittlement at room temperature and a low stress rupture strength at 1500° F. Silicon as described above, is desirable in some small amounts as a deoxidizing agent and for improving castability and weldability of the alloy.

Phosphorous is not required. However, when used in amount up to 0.1% and in the absence of nitrogen, improves the room temperature and high temperature properties of the alloy in the as cast condition. This will be evident by a comparison of the properties of alloys No. 3, 9, 10, and 8 and of alloys 5 and 13.

Additions of boron in amounts up to 0.2% as shown by alloys 3A, 3B, 3C and 3D appear to improve the stress-rupture strength at 1500° F. as evident from a comparison with alloy 3. Above this concentration with this base composition no further improvement was evident. Moreover, increasing amounts within the range up to 0.2% gave a slight improvement in hot strength but recorded a substantial drop in cold ductility when above 0.02 concentration, the elongation then decreasing from 4% to 1% when the boron content was 0.2. Addition of 1.0% boron in compositions having a lower total of carbide formers as in example 136 also improved the stress rupture strength but produced a lower value of cold ductility.

Out of the many alloys made in accordance with the teachings of our invention and for which data is recorded in the above table, those preferred by reason of high temperature strength, and room temperature properties are found, for example, in alloys 6 and 15. Alloy 6 in addition to iron and impurities contained substantially 20% Cr, 5% Ni, 5% Mn, 1% Mo, 1% W, 1% Cb, 1% C, and 0.5% Si, and alloy 15 similar amounts of Cr, Ni, Mn, C, and Si, about twice as much of each of Mo, W, and Cb and including between 0.05% to 0.3% N.

These two alloys have been subjected to extensive tests to determine the following properties:

- (1) Short time tensile strength at temperatures up to 1800° F. and stress rupture and creep data at temperatures of 1200° F. to 1500° F.
- (2) Thermal shock behavior as compared to cobalt based so-called "super" alloys.
- (3) Thermal expansion characteristics.
- (4) Oxidation behavior.

- (5) Microstructural characteristics in the as-cast condition.  
 (6) Welding characteristics under restrained and unrestrained conditions.

The short time tensile data is given below in Table III:

TABLE III  
*Short Time Tensile Properties of Alloys 6 and 15*

| Testing Temp. | Alloy 6            |                 |                 | Alloy 15           |                 |                 |
|---------------|--------------------|-----------------|-----------------|--------------------|-----------------|-----------------|
|               | U.T.S.<br>(p.s.i.) | Percent<br>E.L. | Percent<br>R.A. | U.T.S.<br>(p.s.i.) | Percent<br>E.L. | Percent<br>R.A. |
| Room Temp.    | 105,000            | 4.0             | 2.0             | 125,000            | 3.0             | 2.0             |
| 600° F.       | 86,000             | 5.0             | 2.0             |                    |                 |                 |
| 900° F.       | 78,000             | 5.0             | 2.5             | 93,500             | 5.0             | 4.6             |
| 1,200° F.     | 70,000             | 6.0             | 13.0            | 79,000             | 4.0             | 2.0             |
| 1,500° F.     | 41,000             | 18.0            | 20.0            | 63,000             | 12.0            | 13.0            |
| 1,700° F.     | 27,000             | 28.0            | 32.0            | 34,500             | 23.0            | 66.0            |
| 1,800° F.     | 22,400             | 45.0            | 73.0            | 26,850             | 52.0            | 60.0            |

From this short time tensile data it is apparent that alloy 15 is much stronger than alloy 6 over the temperature range recorded. On the other hand, alloy 6 is possessed of a higher degree of ductility at room temperature.

The stress-rupture strengths for alloys 6, 12, and 15 and of the cobalt base alloys HS21 and HS31 at elevated temperatures are given in Table IV below:

TABLE IV  
*Stress Rupture Characteristics of Alloys 6 and 15 at High Temperature as Compared to Cobalt-Base Alloys HS31 and HS21<sup>1</sup>*

| Alloy | Temp.<br>(° F.) | Stress,<br>p.s.i. | Time,<br>Hours | 100-hour<br>Stress<br>Rupture,<br>p.s.i. | Percent<br>Elonga-<br>tion |
|-------|-----------------|-------------------|----------------|------------------------------------------|----------------------------|
| 6     | 1,200           | 55,000            | 1,571          | 67,000                                   | 5.0                        |
|       |                 | 65,000            | 113.6          |                                          | 7.0                        |
|       |                 | 67,500            | 77.9           |                                          | 8.5                        |
|       | 1,300           | 45,000            | 386.6          | 51,000                                   | 7.0                        |
|       |                 | 50,000            | 148.3          |                                          | 9.0                        |
|       |                 | 55,000            | 36.4           |                                          | 7.0                        |
|       | 1,400           | 30,000            | 323.3          | 34,000                                   | 14.5                       |
|       |                 | 37,500            | 41.4           |                                          | 18.0                       |
|       |                 | 45,000            | 5.2            |                                          | 14.0                       |
|       | 1,500           | 20,000            | 1,215.0        | 27,000                                   | 4.5                        |
| 15    |                 | 22,500            | 590.0          |                                          | 45                         |
|       |                 | 25,000            | 305.0          |                                          |                            |
|       |                 | 27,500            | 125.0          |                                          |                            |
|       | 1,200           | 30,000            | 24.5           |                                          |                            |
|       |                 | 55,000            | 901.1          | 67,500                                   | 8.0                        |
|       |                 | 60,000            | 295.0          |                                          | 6.5                        |
|       |                 | 70,000            | 70.3           |                                          | 6.0                        |
|       | 1,300           | 45,000            | 252.2          | 50,500                                   | 20.0                       |
|       |                 | 52,500            | 67.4           |                                          | 12.0                       |
|       |                 | 65,000            | 7.0            |                                          | 9.0                        |
| 12    | 1,400           | 30,000            | 270.7          | 34,000                                   | 18.0                       |
|       |                 | 37,500            | 45.4           |                                          | 25.0                       |
|       |                 | 42,500            | 20.1           |                                          | 17.0                       |
|       | 1,500           | 25,000            | 275.5          | 27,000                                   | 12.0                       |
|       |                 | 27,500            | 111.0          |                                          | 17.0                       |
|       |                 | 30,000            | 37.0           |                                          | 16.0                       |
|       | 1,700           | 15,000            | 127.5          |                                          | 3.0                        |
|       | HS21            | 1,200             |                | 51,000                                   |                            |
|       |                 | 1,300             |                | 43,000                                   |                            |
|       |                 | 1,400             |                | 24,000                                   |                            |
| HS31  | 1,500           |                   |                | 22,000                                   |                            |
|       | 1,700           |                   |                | 13,000                                   |                            |
|       | 1,200           |                   |                | 55,000                                   |                            |
|       | 1,300           |                   |                | 46,000                                   |                            |
|       | 1,400           |                   |                | 36,000                                   |                            |
|       | 1,500           |                   |                | 28,000                                   |                            |
|       | 1,700           |                   |                | 17,000                                   |                            |

<sup>1</sup> Values for HS31 and HS21 as reported in "Haynes Alloys," published by Haynes Stellite Company (Division of Union Carbide and Carbon Corporation).

<sup>2</sup> Heat-treated condition.

It will be apparent that the creep-rupture strengths of iron base alloys 6 and 15 are much superior to the cobalt base alloy HS21 over the entire range of temperatures tested and superior to HS31 at temperatures up to 1400° F. and substantially equivalent in the temperature range of 1400° F. to 1500° F.

The oxidation resistance of alloys 6 and 15 and cobalt alloy HS31 were evaluated at temperatures of 1500° F.,

1800° F., and 2000° F. Cycling oxidation tests as well as continuous exposures in still air were made. The results based upon weight loss indicate that both of alloys 6 and 15 have comparable refractory characteristics at elevated temperatures up to about 1500° F. but their oxidation resistance is not as great as cobalt base alloy HS31 at 1800° F. and above. The scaling temperatures of these iron base alloys 6 and 15 is in the order of 1800° F. which is comparable to other types of stainless steels containing about 20% chromium.

The welding characteristics of iron base austenitic alloys such as alloys 6 and 15 indicate many advantages. Studies show that sound and good weldments can be obtained in both restrained and unrestrained conditions and without the preheating and post heating treatments required on other alloys such as HS31. The latter cobalt base alloys must be preheated to about 600° F. prior to welding. Unless this is done, stresses created provide cracking in the joints and other portions of the welded parts. After welding HS31, parts must be post heated to 1200° F. to release welding stresses.

Alloys of our invention such as alloys 6 and 15 do not require these operations to be welded. No adverse effects are noted by visual, X-ray and radiographic examinations where such steps were eliminated. Although the reason therefor is not definitely known, it is believed that the presence of silicon in these alloys accounts to a substantial degree for their improved weldability and improved ductility.

Alloys 6 and 15 have been welded in the unrestrained condition using commercially available alloy welding rods such as "19/9 W-Mo" (a stainless steel base alloy), "L-605" (a cobalt base alloy) and "N-155" (a cobalt-nickel rich iron base alloy). Turbine wheel ring blades of alloy 6 were welded (a restrained weld) to a "16-25-6" stainless steel alloy hub using a "19/9 W-Mo" filler rod and by operations using a 600° F. preheat and 1200 F. post treatment and by operations omitting these preheat and post heating steps with equal effect.

The welds are good. There is no tendency toward cracking of these alloys 6 and 15 during welding in a restrained condition. This is especially significant. Moreover, the material flows well and shows a good heat-affected zone microstructurally. There was little if any difference noted in welding with various rods used for unrestrained welds.

The iron base alloys of our invention, as previously described, are austenitic. They furthermore contain in addition to other types of compounds which are also precipitated in the solid solution matrix, one or more of the primary or massive, ledeburite or eutectic and spheroidal or dot-type types of carbides. Photomicrographs of metallographic specimens of a composition such as alloy 3 showed that this alloy in the as-cast condition consists of an austenitic matrix embedding dot-like carbides randomly distributed and a continuous interdendritic network comprising both ledeburite and massive carbides. The ledeburite network is believed to consist mainly of a mixture of complex carbides of chromium, molybdenum, tungsten and columbium carbides with austenite. The hard massive "cross" carbides of the secondary phases are quite typical of columbium carbide while the fine spheroidal precipitate randomly distributed within the matrix have been identified as  $M_{23}C_6$  complex carbides.

Photomicrographic study of alloys 6 and 15 i.e., the preferred alloys, show a much more balanced alloy structure than those discussed above in terms of distribution and relative amounts of secondary phases. Our studies also make it appear that optimum stress-rupture strength in the alloys of our invention is dependent upon a microstructural equilibrium between solid solution matrix composition, primary and eutectic carbides, available carbon and carbide forming elements and available nitrogen and nitride formers for matrix strengthening as well as proper

partition of the strengtheners between secondary phases and matrix.

Although the functions of the alloying elements in the complex austenitic iron base compositions of our invention are imperfectly understood, certain characteristics may bear restating.

(a) The high temperature properties of our alloys depend upon both solid solution and precipitation hardening.

(b) Critical quantities of minor elements when present affect the microstructural aspects of the composition and aid in obtaining elevated temperature properties.

(c) A stable F.C.C. iron matrix is essential that is relatively lean in austenite forming elements of the non-strengthening type such as nickel to accommodate the addition of optimum amounts of strengtheners without overstraining the iron lattice at both room and elevated temperatures.

(d) For best properties an iron solid solution is essential containing multiple amounts of soluble and insoluble strengthening elements of the NaCl-type of cubic carbide formers critically balanced with the carbon content and distributed randomly within the matrix structure and forming a distinctive network at the grain boundaries.

(e) The alloy will be an iron base alloy capable of holding an optimum amount of dissolved and combined nitrogen which may be present in controlled concentration and balanced to the total amounts of nitride formers (chromium, manganese, and columbium).

(f) An iron base solid solution is required containing enough free or uncombined chromium to provide adequate oxidation resistance at elevated temperatures.

From the foregoing description and discussion of the features of our invention, it will be apparent that we have produced iron base alloys of improved high temperature character which provide advantageous combination of mechanical properties at both room and elevated temperatures approaching those of the cobalt base alloys, for example HS31. Moreover, in order to retain a structurally stable austenitic matrix providing good hot strength, the basic composition of the alloys of our invention must be within close limits of chemistry. Thus the nickel content for optimum results will preferably be above about 2% and preferably at the 5% level. Manganese additions when used at about the 5% level serve as strengtheners in the forming of nitrides as well as austenite stabilizing when dissolved in the iron lattice. Critical amounts of carbon in amounts of about 0.9% to 1.1% are preferred for optimum creep rupture strength and for adequate oxidation resistance the chromium content will preferably be in order of 15 to 20%. Moreover, the basic strengthening mechanism at elevated temperatures in certain alloys, for instance in preferred alloy 6, was derived from carbide phases and in other cases for example preferred alloy 15, was derived from both carbide and nitride phase. Furthermore of all the NaCl-type of carbide forming elements, tungsten, molybdenum and columbium in triple combination were found to be the most potent strengtheners. These gave optimum high temperature properties when used approximately in the proportion of 1:1:1 by weight and accomplished this at several different levels of concentration. Alloy 15 which contained a total of about 6% of strengtheners i.e., about 2% each of W, Mo, and Cb and also contained 0.05% to 0.3% nitrogen gave the best combination of properties at both room and elevated temperatures. Alloy 6 which contained about a 3% total of strengtheners i.e., about 1% each of W, Mo, and Cb possessed superior cold tensile ductility but lower hot tensile strength.

Although the present invention has been described in conjunction with preferred embodiments, it is to be understood that modifications and variations may be resorted to without departing from the spirit and scope of the invention, as those skilled in the art will readily understand. Such modifications and variations are considered to be

within the purview and scope of the invention and appended claims.

This application is a continuation-in-part of our application Serial No. 815,252, filed May 25, 1959.

We claim:

- 5 1. An iron base casting type alloy for producing products of complex shape and having substantial oxidation resistance and high strength at elevated temperatures, said alloy consisting essentially of by weight percent, about 0.8 to 1.6% carbon; about 12 to 35% chromium; between 0 to 2.5% silicon; between 0.2 to 12% of a plurality of carbide forming elements from the group consisting of tungsten in the range 0.1 to 10%, molybdenum in the range 0.1 to 9%, columbium and tantalum, said columbium and tantalum combined being in the range 0.1 to 5%; up to about 15% of metal from the group consisting of, nickel in the range 0 to about 8%, manganese in the range 0 to 15%, and cobalt in the range 0 to 8%; and from 0 to 0.6% nitrogen; the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero; said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 10 2. An iron base casting type alloy as claimed in claim 1 wherein the carbide forming elements are present in amount above 3% and nitrogen is present in amount between about 0.05 and 0.3%.
- 15 3. An iron base casting type alloy as claimed in claim 1 including between 0 to 2% titanium, 0 to 5.0% vanadium, 0 to 1% boron, 0 to 0.2% phosphorus, and up to 1% in the aggregate of contaminants including zirconium and wherein the 100 hour stress rupture strength at 1500° F. is at least about 19,000 p.s.i.
- 20 4. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 25 5. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 30 6. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 35 7. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 40 8. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 45 9. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 50 10. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 55 11. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 60 12. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 65 13. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.
- 70 14. An iron base casting type alloy for producing products of complex shape and having substantial oxidation resistance and high strength at elevated temperatures, said alloy consisting essentially of by weight percent, about 0.8 to 1.25% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range 0.1 to 5%; up to about 15% of metal from the group consisting of, nickel in the range 0 to 8%, manganese in the range 0 to 15%, and cobalt in the range 0 to 8%, and from 0 to 0.6% nitrogen, the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

5. An iron base casting type alloy for producing products of complex shape and having substantial oxidation resistance and high strength at elevated temperatures, said alloy consisting essentially of by weight percent, above about 1% up to about 1.1% carbon; about 12 to 35% chromium; between 0 to 2.5% silicon; between 0.2 to 12% of a plurality of carbide forming elements from the group consisting of tungsten in the range 0.1 to 10%, molybdenum in the range 0.1 to 9%, columbium and tantalum, said columbium and tantalum combined being in the range 0.1 to 5%; up to about 15% of metal from the group consisting of, nickel in the range 0 to 15%, manganese in the range 0 to 8%, and cobalt in the range 0 to 8%; and from 0 to 0.6% nitrogen; the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero; said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

6. An iron base casting type alloy for producing products of complex shape and having substantial oxidation resistance and high strength at elevated temperatures, said alloy consisting essentially of by weight percent, above about 0.9% up to about 1.1% carbon; about 12 to 25% chromium; between 0 to 2.5% silicon; between 0.2 to 9% of a plurality of carbide forming elements from the group consisting of tungsten in the range 0.1 to 8.5%, molybdenum in the range 0.1 to 8.5%, columbium and tantalum, said columbium and tantalum combined being in the range of 0.1 to 5%; up to about 15% of metal from the group consisting of, nickel in the range 0 to 15%, manganese in the range 0 to 8%, and cobalt in the range 0 to 8%; and from 0 to 0.6% nitrogen; the balance essentially iron, said iron content being at least 40%, said nickel being at least about 2% when said manganese is less than about 1%, said manganese being at least 2 to 10% when the nickel is less than 2% and nitrogen is present, at least between about 5 to 10% when substantially no nitrogen is present and the nickel is less than about 2%, and at least about 10% when the nickel is zero; said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

7. An iron base casting type alloy for producing products of complex shape and having substantial oxidation resistance and high strength at elevated temperatures, said alloy consisting essentially of by weight percent, above about 0.9 up to about 1.1% carbon; about 12 to 25% chromium; between 0 to 2.5% silicon; between 0.6 to 9% of carbide forming elements consisting of tungsten in the range 0.2 to 6.0%, molybdenum in the range 0.2 to 7.0%, and 0.2 to 4% of metal selected from the group consisting of columbium and tantalum; up to about 15% of metal from the group consisting of, nickel in the range 0 to 8%, manganese in the range 0 to 15%, and cobalt in the range 0 to 8%; and from 0 to 0.6% nitrogen; the balance essentially iron, said iron content being at least

5 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero; said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

20 8. An iron base casting type alloy for producing products of complex shape and having substantial oxidation resistance and high strength at elevated temperatures in the order of 1500° F., said alloy consisting essentially of by weight percent, about 0.9 to 1.1% carbon, about 12 to 25% chromium, about 0.2 to 7% molybdenum, about 0.2 to 6% tungsten, about 0.2 to 4% of metal from the group consisting of columbium and tantalum, said molybdenum, tungsten, columbium and tantalum combined not exceeding about 9%, up to about 15% of metal from the group consisting of nickel in the range of about 2 to 8%, manganese in the range of 0 to about 9% and cobalt in the range of 0 to about 8% with the nickel and manganese combined not exceeding about 11%, the balance essentially iron, said iron content being at least 40%, said alloy being austenitic at room temperatures and being characterized in the as cast condition by a tensile strength of at least 80,000 p.s.i. and at least about 2% elongation at atmospheric temperature, a hot strength of at least 40,000 p.s.i. and less than 35% elongation at 1500° F. and a 100 hour rupture strength at 1500° F. of at least 24,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

30 9. An iron base casting type alloy for producing products of complex shape and having substantial oxidation resistance and high strength at elevated temperatures in the order of 1500° F., said alloy consisting essentially of by weight percent, about 0.8 to 1.25% carbon, about 0.1 to 2% silicon, about 18 to 22% chromium, about 0.5 to 3% molybdenum, about 0.3 to 5% tungsten, about 0.5 to 2% of metal from the group consisting of columbium and tantalum, said molybdenum, tungsten, columbium and tantalum combined not exceeding about 9%, up to about 15% of metal from the group consisting of nickel in the range of about 2 to 6%, manganese in the range of 0 to about 7% and cobalt in the range of 0 to about 8% with the nickel and manganese combined not exceeding about 11%, the balance essentially iron, said iron content being at least 40%, said alloy being austenitic at room temperatures and being characterized in the as cast condition by a tensile strength of at least 80,000 p.s.i. and at least about 2% elongation at atmospheric temperature, a hot strength of at least 40,000 p.s.i. and less than 35% elongation at 1500° F. and a 100 hour rupture strength at 1500° F. of at least 22,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

40 10. An iron base casting type alloy for producing products of complex shape and having substantial oxidation resistance and high strength at elevated temperatures in

the order of 1500° F., said alloy consisting essentially of by weight percent, about 0.8 to 1.25% carbon, about 0.1 to 2% silicon, about 18 to 22% chromium, up to 0.3% nitrogen, about 0.5 to 3% molybdenum, about 0.5 to 3% tungsten, about 0.5 to 2% of metal from the group consisting of columbium and tantalum, about 2 to 6% nickel, up to about 7% manganese, the nickel and manganese combined not exceeding about 11%, the balance essentially iron, said iron content being at least 60%, said alloy being austenitic at room temperatures and being characterized in the as cast condition by a tensile strength of at least 80,000 p.s.i. and at least about 2% elongation at atmospheric temperature, a hot strength of at least 40,000 p.s.i. and less than 35% elongation at 1500° F. and a 100 hour rupture strength at 1500° F. of at least 22,000 p.s.i. and said alloy being castable into complex shapes and being machinable and weldable, a test bar thereof  $\frac{1}{4}$ " in diameter exposed to 1500° F. for 100 hours being generally characterized by a structure having an interdendritic network of substantially ledeburite phases outlining and austenitic phase embedding relatively fine dot-like precipitates randomly distributed therein.

11. An iron base casting type alloy having substantial oxidation resistance and high strength at elevated temperatures, said alloy consisting essentially of by weight percent, about 0.8 to 1.4% carbon, about 18 to 22% chromium, about 2 to 6% nickel, about 1.0 to 2.0% molybdenum, about 1.0 to 2.0% tungsten, about 1.0 to 2% of metal from the group consisting of columbium and tantalum, from 0 to 7% manganese, from 0 to 0.6% nitrogen, about 0.4 to 2% silicon the balance essentially iron, said iron content being between about 60 to 75%, said alloy being austenitic at atmospheric temperature and characterized in the as cast condition by a tensile strength of at least 90,000 p.s.i. at atmospheric temperature, a hot strength of at least 40,000 p.s.i. with less than 35% elongation at 1500° F. and a 100 hour rupture strength at 1500° F. of at least 20,000 p.s.i. and said alloy being castable into complex shapes and being machinable and weldable and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

12. An iron base casting type alloy having substantial oxidation resistance and high strength at elevated temperatures in the order of 1500° F., said alloy consisting essentially of by weight percent, about 0.8 to 1.25% carbon, about 2 to 8% nickel, about 12 to 25% chromium, substantially equal amounts between about 1 to 2% each of molybdenum, tungsten and metal selected from the group consisting of columbium and tantalum, up to about 9% manganese, the balance essentially iron, said iron content being between about 60 to 75%, said nickel and manganese combined being not more than 15%, said alloy being austenitic at atmospheric temperatures and characterized in the as cast condition by a tensile strength of at least 90,000 p.s.i. and at least 2% elongation at atmospheric temperatures, a hot strength of at least 40,000 p.s.i. with less than 35% elongation at 1500° F. and a 100 hour rupture strength at 1500° F. of at least 22,000 p.s.i., and said alloy being castable into complex shapes and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

13. An iron base casting type alloy capable of withstanding severe stress at high temperatures in the order of 1500° F., said alloy consisting essentially of by weight percent, about 1% carbon, about 20% chromium, about 5% nickel, about 4.5 to 5% manganese, about 1 to 2% columbium, from 0 to 0.3% nitrogen, and about 0.1 to 0.5% silicon, the balance essentially iron, said iron content being at least about 60%, said alloy being austenitic at room temperature and characterized in the as cast condition by a 100 hour rupture strength at 1500° F. of at least about 22,000 p.s.i., and said alloy being castable

1.25% molybdenum, about 1% tungsten, about 1% columbium and about 0.5 to 1.25% silicon, the balance essentially iron, said iron content being between about 60 to 75%, said alloy being austenitic at room temperature and characterized in the as cast condition by a 100 hour rupture strength at 1500° F. of at least about 27,000 p.s.i., and said alloy being castable into complex shapes and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

14. An iron base casting type alloy capable of withstanding severe stress at high temperatures in the order of 1500° F., said alloy consisting essentially of by weight percent, about 1% carbon, about 20% chromium, about 5% nickel, about 4.5 to 5% manganese, about 2% molybdenum, about 1.75 to 2% tungsten, about 2 to 2.5% columbium, about 0.5% silicon, and about 0.05 to 0.3% nitrogen, the balance essentially iron, said iron content being between about 60 to 75%, said alloy being austenitic at room temperature and characterized in the as cast condition by a 100 hour rupture strength at 1500° F. of at least about 27,000 p.s.i., and said alloy being castable into complex shapes and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

15. An iron base casting type alloy capable of withstanding severe stress at high temperatures in the order of 1500° F., said alloy consisting essentially of by weight percent, about 1% carbon, about 20% chromium, about 2% nickel, about 2% molybdenum, about 2% tungsten, about 2% columbium, about 0.3% nitrogen and about 0.5% silicon, the balance essentially iron, said iron content being at least about 60%, said alloy being austenitic at room temperature and characterized in the as cast condition by a 100 hour rupture strength at 1500° F. of at least about 22,000 p.s.i., and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

16. An iron base casting type alloy capable of withstanding severe stress at high temperatures in the order of 1500° F., said alloy consisting essentially of by weight percent, about 1% carbon, about 20% chromium, about 2 to 10% manganese, about 2% molybdenum, about 2% tungsten, about 2% columbium, about 0.5% silicon, and about 0.2 to 0.5% nitrogen, the balance essentially iron, said iron content being at least about 60%, said alloy being austenitic at room temperature and characterized in the as cast condition by a 100 hour rupture strength at 1500° F. of at least about 20,000 p.s.i., and said alloy being castable into complex shapes and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

17. An iron base casting type alloy capable of withstanding severe stress at high temperatures in the order of 1500° F., said alloy consisting essentially of by weight percent, about 0.9 to 1.1% carbon, about 15 to 20% chromium, about 2 to 5% nickel, about 1 to 4% molybdenum, about 1 to 2% tungsten, about 1 to 2% columbium, from 0 to 0.3% nitrogen, and about 0.1 to 0.5% silicon, the balance essentially iron, said iron content being at least about 60%, said alloy being austenitic at room temperature and characterized in the as cast condition by a 100 hour rupture strength at 1500° F. of at least about 22,000 p.s.i., and said alloy being castable

into complex shapes and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

18. An iron base casting type alloy capable of withstanding severe stress at high temperatures in the order of 1500° F., said alloy consisting essentially of by weight percent, about 0.9 to 1.1% carbon, about 20% chromium, about 5% nickel, about 5% manganese, about 4 to 6% of metal from the group molybdenum, tungsten, columbium and tantalum, about 0.1 to 0.5% silicon, and about 0.05 to 0.6% nitrogen, the balance essentially iron, said iron content being at least about 60%, said alloy being austenitic at room temperature and characterized in the as cast condition by a 100 hour rupture strength at 1500° F. of at least about 22,000 p.s.i., and said alloy being castable into complex shapes and a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

19. An iron base casting type alloy having substantial oxidation resistance and high strength at high temperature and being substantially free of cobalt, said alloy consisting essentially of by weight percent, about 0.8 to 1.25% carbon, about 12 to 25% chromium, less than 2% nickel, between about 1 to 2% each of tungsten, molybdenum and metal from the group consisting of columbium and tantalum, at least 2% and under 15% manganese and at least 0.2% and under 0.6% nitrogen, the balance essentially iron, said iron content being at least 60%, said alloy being austenitic at room temperature and being characterized in the as cast condition by a 100 hour rupture strength at 1500° F. of at least 18,000 p.s.i., a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

20. An iron base casting type alloy having substantial oxidation resistance and high strength at elevated temperatures, said alloy consisting essentially of by weight percent, about 0.65 to 1.25% carbon, about 18 to 22% chromium, about 2 to 6% nickel, about 1.0 to 3.0% molybdenum, about 1.0 to 3.0% tungsten, about 1.0 to 2% of metal from the group consisting of columbium and tantalum, from 0 to 7% manganese, from 0.1 to 0.6% nitrogen, about 0.4 to 2% silicon, the balance essentially iron, said iron content being between about

60 to 75%, said alloy being austenitic at atmospheric temperature and characterized in the as cast condition by a tensile strength of at least 90,000 p.s.i. at atmospheric temperature, a hot strength of at least 40,000 p.s.i. with less than 35% elongation at 1500° F. and a 100 hour rupture strength at 1500° F. of at least 20,000 p.s.i. and said alloy being castable into complex shapes and being machinable and moldable, a test bar thereof  $\frac{1}{4}$ " in diameter exposed to 1500° F. for 100 hours being generally characterized by a structure having an interdendritic network of substantially ledeburite and nitride phases outlining an austenitic phase embedding relatively fine dot-like precipitates randomly distributed therein.

21. An iron base casting type alloy for producing products of complex shape and having substantial oxidation resistance and high strength at elevated temperatures, said alloy consisting essentially of, by weight percent, about 0.8 to 1.6% carbon; about 12 to 35% chromium; between 0 to 2.5% silicon; between 0.2 to 12% of a plurality of carbide forming elements from the group consisting of tungsten in the range 0.1 to 10%, molybdenum in the range 0.1 to 9%, columbium and tantalum, said columbium and tantalum combined being in the range 0.1 to 5%; up to about 15% of metal from the group consisting of, nickel in the range 0 to 15%, manganese in the range 0 to 15%, and cobalt in the range 0 to 8% and from 0 to 0.6% nitrogen; the balance essentially iron, said iron content being at least 40%, said nickel being at least about 2% when said manganese is less than about 1%, said manganese being at least between 2 to 10% when the nickel is less than 2% and nitrogen is present, at least between about 5 to 10% when substantially no nitrogen is present and the nickel is less than about 2%, and at least about 10% when the nickel is zero; said alloy being substantially free of vanadium, said alloy being austenitic at room temperature and being characterized in the as cast condition by a 100 hour rupture strength at 1500° F. of at least about 20,000 p.s.i. and said alloy being castable into complex shapes and products, a test bar thereof  $\frac{1}{4}$ " in diameter exposed to 1500° F. for 100 hours being generally characterized by a structure having an interdendritic network of substantially ledeburite phases outlining an austenitic phase embedding relatively fine dot-like precipitates randomly distributed therein.

45 References Cited in the file of this patent

UNITED STATES PATENTS

|           |        |               |
|-----------|--------|---------------|
| 2,380,854 | Lorig  | July 31, 1945 |
| 2,429,800 | Briggs | Oct. 28, 1947 |

50 FOREIGN PATENTS

|         |               |               |
|---------|---------------|---------------|
| 647,701 | Great Britain | Dec. 20, 1950 |
| 160,713 | Australia     | Feb. 24, 1955 |